



US007981270B2

(12) **United States Patent**  
**Rosenbaum et al.**

(10) **Patent No.:** **US 7,981,270 B2**  
(b4) **Date of Patent:** **\*Jul. 19, 2011**

(54) **EXTRA LIGHT HYDROCARBON LIQUIDS**

(75) Inventors: **John M. Rosenbaum**, Richmond, CA (US); **Brent K. Lok**, San Francisco, CA (US); **Joseph M. Pudlak**, Vallejo, CA (US)

(73) Assignee: **Chevron U.S.A. Inc.**, San Ramon, CA (US)

(\*) Notice: Subject to any disclaimer, the term of this patent is extended or adjusted under 35 U.S.C. 154(b) by 1557 days.

This patent is subject to a terminal disclaimer.

(21) Appl. No.: **11/353,205**

(22) Filed: **Feb. 14, 2006**

(65) **Prior Publication Data**

US 2006/0201852 A1 Sep. 14, 2006

**Related U.S. Application Data**

(60) Provisional application No. 60/660,464, filed on Mar. 11, 2005.

(51) **Int. Cl.**

**C10G 71/00** (2006.01)

**C10M 105/04** (2006.01)

(52) **U.S. Cl.** ..... **208/18**; 208/19; 208/950; 508/110; 508/469; 508/591

(58) **Field of Classification Search** ..... 208/18, 208/19, 950; 508/110, 469, 591

See application file for complete search history.

(56) **References Cited****U.S. PATENT DOCUMENTS**

|                 |         |                             |
|-----------------|---------|-----------------------------|
| 3,773,650 A     | 11/1973 | Hislop et al.               |
| 3,775,288 A     | 11/1973 | Eagen et al.                |
| 3,852,207 A     | 12/1974 | Stangeland et al.           |
| 3,904,513 A     | 9/1975  | Fischer et al.              |
| 4,157,294 A     | 6/1979  | Iwao et al.                 |
| 4,347,121 A     | 8/1982  | Mayer et al.                |
| 4,440,871 A     | 4/1984  | Lok et al.                  |
| 4,477,333 A     | 10/1984 | Hafez                       |
| 4,568,663 A     | 2/1986  | Mauldin                     |
| 4,673,487 A     | 6/1987  | Miller                      |
| 4,810,357 A     | 3/1989  | Chester et al.              |
| 4,943,424 A     | 7/1990  | Miller                      |
| 5,135,638 A     | 8/1992  | Miller                      |
| 5,158,665 A     | 10/1992 | Miller                      |
| 5,282,958 A     | 2/1994  | Santilli et al.             |
| 6,008,164 A *   | 12/1999 | Aldrich et al. .... 508/110 |
| 6,017,859 A     | 1/2000  | Rossi et al.                |
| 6,096,691 A     | 8/2000  | Conary et al.               |
| 6,235,688 B1    | 5/2001  | Small et al.                |
| 6,271,184 B1    | 8/2001  | Seebauer et al.             |
| 6,544,935 B1    | 4/2003  | Vargo et al.                |
| 6,689,723 B2    | 2/2004  | Sullivan et al.             |
| 6,703,353 B1 *  | 3/2004  | Lok et al. .... 508/110     |
| 7,018,962 B2    | 3/2006  | Bloch et al.                |
| 2004/0077505 A1 | 4/2004  | Daniel et al.               |
| 2004/0094453 A1 | 5/2004  | Lok et al.                  |
| 2004/0178118 A1 | 9/2004  | Rosenbaum et al.            |
| 2004/0254082 A1 | 12/2004 | Bloch et al.                |

|                   |         |                       |         |
|-------------------|---------|-----------------------|---------|
| 2005/0098476 A1 * | 5/2005  | Miller .....          | 208/19  |
| 2005/0133407 A1   | 6/2005  | Abernathy et al.      |         |
| 2005/0133408 A1   | 6/2005  | Abernathy et al.      |         |
| 2005/0133409 A1   | 6/2005  | Abernathy et al.      |         |
| 2005/0261147 A1 * | 11/2005 | Rosenbaum et al. .... | 508/466 |
| 2006/0172898 A1 * | 8/2006  | Roby et al. ....      | 508/485 |

**FOREIGN PATENT DOCUMENTS**

|    |                  |        |
|----|------------------|--------|
| EP | 0 609 079 A1     | 1/1994 |
| EP | 0 776 959 A2     | 6/1997 |
| EP | 0 668 342 B1     | 8/1999 |
| EP | 1 452 579 A1     | 9/2004 |
| WO | 99/20720 A1      | 4/1999 |
| WO | 99/41332 A1      | 8/1999 |
| WO | 99/41335 A1      | 8/1999 |
| WO | 00/14179 A1      | 3/2000 |
| WO | 00/14183 A1      | 3/2000 |
| WO | 00/14187 A2      | 3/2000 |
| WO | 00/14188 A2      | 3/2000 |
| WO | 02/064710 A2     | 8/2002 |
| WO | WO02/064710 A2 * | 8/2002 |
| WO | 02/070627 A1     | 9/2002 |
| WO | 02/070629 A1     | 9/2002 |
| WO | 02/070631 A2     | 9/2002 |
| WO | 2005/066314      | 7/2005 |

**OTHER PUBLICATIONS**

U.S. Appl. No. 11/353,035 "Processes for Producing Extra Light Hydrocarbon Liquids", Rosenbaum et al., filed Feb. 14, 2006.

ILSAC GF-4 Standard for Passenger Car Engine Oils , International Lubricant Standardization and Approval Committee, Japan Automobile Manufacturers Association, DaimlerChrysler Corporation, Ford Motor Company and General Motors Corporation, (2004).

Anderson, et al., "Reactions on ZSM-5-Type ZeoliteCatalyst", *J. of Catalysis* 58:114-130 (1979).

Baerlocher, Ch., Meier, W.M., and Olson, D.H., *Atlas of Zeolite Framework Types*, Fifth Revised Edition, Elsevier, pp. 10-15 (2001).

Barrer, R.M., *Zeolites, Science and Technology*, F.R. Rodrigues, L.D. Rollman and C. Naccache, editors, *NATO ASI Series* p. 75 (1984).

Gatto, V.J., et al., "The Influence of Chemical Structure on the Physical Properties and Antioxidant Response of Hydrocracked Base Stocks and Polyalphaolefins", *J. Synthetic Lubrication* 19(1):3-18 (2002).

(Continued)

*Primary Examiner* — Ellen M McAvoy

*Assistant Examiner* — Latosha Hines

(74) *Attorney, Agent, or Firm* — Merchant & Gould

(57) **ABSTRACT**

The present invention relates to an extra light hydrocarbon liquid derived from highly paraffinic wax. This extra light hydrocarbon liquid is suitable for use as a lubricant additive diluent oil in oil soluble additive concentrates. This extra light hydrocarbon liquid derived from highly paraffinic wax has a viscosity of between about 1.0 and 3.5 cSt at 100° C. and a Noack volatility of less than 50 weight % and comprises greater than 3 weight % molecules with cycloparaffinic functionality and less than 0.30 weight percent aromatics. The extra light hydrocarbon liquid makes an excellent lubricant additive diluent oil because it has low volatility, low viscosity, good additive solubility, and excellent solubility in lubricant base oil stocks. The present invention also relates to finished lubricants comprising the oil soluble additive concentrates made with the extra light hydrocarbon liquid and finished lubricants comprising the oil soluble additive concentrates. The present invention further relates to processes for making

these lubricant additive diluent oils, oil soluble additive concentrates, and finished lubricants.

**43 Claims, No Drawings**

OTHER PUBLICATIONS

*Chemical Technology of Petroleum*, 3<sup>rd</sup> Edition, William Gruse and Donald Stevens, McGraw-Hill Book Company, Inc. New York, pp. 566-570 (1960).

Henderson, H. Ernest, "The North American Basestock Revolution", *Lubricants World*, Sep./Oct. 2004 pp. 12-15.

Kramer, D.C., et al., "Influence of Group II & III Base Oil Composition on VI and Oxidation Stability," presented at the 1999 AIChE Spring National Meeting in Houston, Mar. 16, 1999.

Netherlands Search Report dated Jan. 2, 2007.

\* cited by examiner

## 1

## EXTRA LIGHT HYDROCARBON LIQUIDS

This application claims priority to U.S. Provisional Application Ser. No. 60/660,464, filed Mar. 11, 2005, which is incorporated herein by reference in its entirety.

## FIELD OF THE INVENTION

The present invention relates to a lubricant additive diluent oils derived from highly paraffinic wax and oil soluble additive concentrates comprising this lubricant additive diluent oil. The present invention also relates to finished lubricants comprising the oil soluble additive concentrates. The present invention further relates to processes for making these lubricant additive diluent oils, oil soluble additive concentrates, and finished lubricants.

## BACKGROUND OF THE INVENTION

Lubricant additives, especially automotive additives such as viscosity index improvers and detergent-inhibitor (DI) packages require lubricant additive diluent oils to make them useable. Accordingly, lubricant additive diluent oils are used to dissolve lubricant additives to provide oil soluble additive concentrates. These oil soluble additive concentrates make the additives easier to transport, handle, and ultimately blend into lubricant base oils to provide a finished lubricant. The oil soluble additive concentrates are not useable or suitable as finished lubricants on their own. Rather, the oil soluble additive concentrates are blended with lubricant base oil stocks to provide a finished lubricant. It is desired that the lubricant additive diluent oils readily solubilize the lubricant additive and provide an oil additive concentrate that is readily soluble in the lubricant base oil stocks. In addition, it is desired that the lubricant additive diluent oils not introduce any undesirable characteristics, including, for example, high volatility, high viscosity, and impurities such as heteroatoms, to the lubricant base oil stocks and thus, ultimately to the finished lubricant.

Different lubricant additive diluent oils require differing amounts of lubricant additive diluent oil to provide a suitable oil soluble additive concentrate. By way of example, oil soluble additive concentrates comprising gear oil additive packages may contain as little as 25% weight lubricant additive diluent oil. Oil soluble additive concentrates comprising DI packages typically contain about 50% weight lubricant additive diluent oil. Oil soluble additive concentrates comprising viscosity index improver typically contain about 90% weight or more lubricant additive diluent oil.

Currently, the lubricant additive diluent oils used with most DI packages and viscosity index improvers are highly aromatic base oils that fall into API Group I. API Group I base oils, with their high solvency and good availability, have been preferred as lubricant additive diluent oils. However, these Group I oils have only average to poor low temperature performance, and they are much more susceptible to oxidation than modern oils, which are more highly saturated. In addition, Group I base oils have lower viscosity indexes (VI) and higher volatility than other base oils. Moreover, Group I base oils have high sulfur concentrations. Lubricant additive diluent oils can comprise up to 5 to 10 weight percent of a finished lubricant. Accordingly, the properties of the lubricant additive diluent oils are important as undesirable properties in the lubricant additive diluent oils can negatively impact the properties of the finished lubricant. Although more desirable in terms of their properties for the finished lubricant, conventional API Group II, conventional Group III, and Group IV

## 2

base oils are difficult to use as lubricant additive diluent oils due to their poor ability to solubilize additives. Therefore, these base oils are not practical as lubricant additive diluent oils.

When added to lubricant base oil stocks, typical oil soluble additive, concentrates comprising DI packages or viscosity index improvers, tend to thicken the finished lubricant formulation and impair its low-temperature performance. Low viscosity lubricant additive diluent oils, which have been used in the past in an attempt to avoid thickening the finished lubricant, have either had high volatility or poor additive solubility, making them unsuitable for most applications. When added to engine oils, the typical oil soluble additive concentrates tend to adversely impact the cold-cranking simulator (CCS) viscosity and Mini-Rotary Viscometer (MRV). When added to automatic transmission fluid and gear oils, the typical oil soluble additive concentrates tend to adversely impact the Brookfield Viscosity at low temperature.

Accordingly, lubricant additive diluent oils with low viscosity, low volatility, and low concentrations of impurities, such as sulfur-containing compounds, are desired. Typical lubricant base oils with low volatilities also have high viscosities rendering them unsuitable for most applications, and typical lubricant base oils with low viscosities also have low volatilities and poor additive solubility rendering them unsuitable for most applications.

Engine manufacturers worldwide are introducing chemical limits on engine oils and additives that they believe will provide the safe margins for operation that their exhaust after-treatment hardware requires. These requirements will directly impact what is suitable for use as additives, lubricant base oil stocks, and lubricant additive diluent oils. Low sulfur and phosphorus limits on engine oils are being proposed. At a limit of about 0.3 weight % sulfur, zinc dithiophosphate antiwear additives need to be partially replaced with more costly additives, and reduced sulfur detergents and base oils are needed to provide formulation flexibility. As limits move toward 0.2 weight % sulfur, reduced or zero-sulfur lubricant base oils and diluent oils become essential to meet formulation targets. International Lubricants Standardization and Approval Committee (ILSAC) GF-4 passenger car engine oils, API PC-10 heavy duty engine oil, and other high quality finished lubricant specifications call for low sulfur formulations.

The ILSAC/Oil Committee adopted the new GF-4 specification for passenger car motor oils on Jan. 8, 2004, with a recommended start date for introducing GF-4 into the marketplace of Jul. 1, 2004. A new bench test requirement for engine oils meeting the GF-4 specification are maximum sulfur content by ASTM D 1552. As such, a 10W oil may have a maximum of 0.7 weight % sulfur, while 0W, and 5W oils may have a maximum of 0.5 weight % sulfur. In addition, the oils meeting the GF-4 specification must have a Noack volatility by ASTM D 5800 of less than 15 weight % after one hour at 250° C., and a simulated distillation by ASTM D 6417 with a maximum of 10% at 371° C. API PC-10 is a proposed specification for heavy duty diesel engine oil and is expected to be approved in 2006 or 2007. It is expected that PC-10 oils will also have reduced limits for sulfur, similar to those amounts called for GF-4 passenger car motor oils.

Accordingly, lubricant additive diluent oils with low sulfur, excellent additive solubility, good elastomer compatibility, low volatility, low viscosity, high oxidation stability, good low temperature properties, and excellent solubility in the lubricant base oils are desired.

## SUMMARY OF THE INVENTION

The present invention relates to extra light hydrocarbon liquids derived from highly paraffinic wax. These extra light

hydrocarbon liquids derived from highly paraffinic wax may be used as lubricant additive diluent oils. Accordingly, the present invention relates to lubricant additive diluent oils derived from highly paraffinic wax and oil soluble additive concentrates comprising this lubricant additive diluent oil. The present invention also relates to finished lubricants comprising the oil soluble additive concentrates. The present invention further relates to processes for making these extra light hydrocarbon liquids derived from highly paraffinic wax, the lubricant additive diluent oils, the oil soluble additive concentrates, and the finished lubricants.

#### DETAILED DESCRIPTION OF THE INVENTION

Finished lubricants comprise at least one lubricant base oil and at least one additive. Typically, the at least one additive is added to the lubricant base oil in the form of an oil soluble additive concentrate comprising at least one additive and a lubricant additive diluent oil, to improve the additive's solubility in the lubricant base oil. For lubricant additive diluent oils, it is important that the oil be heavy enough not to contribute volatility to the finished lubricant, but not be so heavy that the oil thickens the finished lubricant.

It has been surprisingly discovered that certain lubricant base oils derived from highly paraffinic wax make excellent lubricant additive diluent oils. Examples of suitable highly paraffinic waxes include Fischer-Tropsch derived wax, slack wax, deoiled slack wax, and refined foots oils, waxy lubricant raffinates, n-paraffin waxes, normal alpha olefin (NAO) waxes, waxes produced in chemical plant processes, deoiled petroleum derived waxes, microcrystalline waxes, and mixtures thereof. These highly paraffinic waxes are processed to provide lubricant base oil fractions having unexpectedly low volatility and low viscosity and unexpectedly also having good additive solubility. In one preferred embodiment, the highly paraffinic wax is a Fischer-Tropsch derived wax and provides a Fischer-Tropsch derived lubricant base oil fraction.

Accordingly, it has been surprisingly discovered that lubricant base oils derived from highly paraffinic wax can advantageously be used as lubricant additive diluent oils, wherein the lubricant base oil comprises greater than 3 weight % molecules with cycloparaffinic functionality and less than 0.30 weight percent aromatics and have kinematic viscosities between about 1.0 cSt and 3.5 cSt at 100° C. and a Noack volatility less than a Noack Volatility Factor as calculated by the following equation:

$$\text{Noack Volatility Factor} = 160 - 40(\text{Kinematic Viscosity at } 100^\circ \text{ C.})$$

Preferably, the lubricant base oil fraction derived from highly paraffinic wax has a viscosity of between about 2.0 and 3.5 cSt at 100° C. and more preferably between about 2.0 and 3.0 cSt at 100° C. Preferably, the lubricant base oil fraction derived from highly paraffinic wax has a Noack volatility of less than 50 weight %. The lubricant base oil fractions derived from highly paraffinic wax according to the present invention have unexpectedly low Noack volatilities given their relatively low kinematic viscosities.

The lubricant base oils of the present invention may also have preferred alkyl branching placements. As such, the lubricant base oils of the present invention may comprise predominantly methyl branching. The branching may be such that there are 6 to 18 alkyl branches per 100 carbon; greater than 25% of the branches are 5 or more carbon atoms apart from each other; and less than 40% of the branches are within 2 to 3 carbon atoms apart from each other.

These lubricant base oils derived from highly paraffinic wax can be used in applications requiring low volatility, low viscosity, exceptional low-temperature performance, and good additive solubility. In addition, these lubricant base oils derived from highly paraffinic wax exhibit excellent oxidation resistance and good elastomer compatibility. Advantageously, the lubricant base oil fractions derived from highly paraffinic wax can be used as additive diluent oils in applications requiring low volatility, such as ILSAC GF-4 and API PC-10 engine oils.

The lubricant base oil fractions derived from highly paraffinic wax of the present invention are prepared from the highly paraffinic wax by a process including hydroisomerization. Preferably, the highly paraffinic wax is hydroisomerized using a shape selective intermediate pore size molecular sieve comprising a noble metal hydrogenation component under conditions of about 600° F. to 750° F.

In one preferred embodiment, the highly paraffinic wax is a Fischer-Tropsch derived wax and provides a Fischer-Tropsch derived lubricant base oil fraction. The lubricant base oil fractions are prepared from the waxy fractions of Fischer-Tropsch syncrude. As such, the Fischer-Tropsch derived lubricant base oil fractions used in the oil soluble additive concentrates are made by a process comprising performing a Fischer-Tropsch synthesis to provide a product stream; isolating from the product stream a substantially paraffinic wax feed; hydroisomerizing the substantially paraffinic wax feed; isolating an isomerized oil; and optionally hydrofinishing the isomerized oil. From the process, a Fischer-Tropsch derived lubricant base oil fraction comprising less than 0.30 weight % aromatics and greater than 3 weight % molecules with cycloparaffinic functionality and having kinematic viscosity between about 1.0 cSt and 3.5 cSt at 100° C. and a Noack volatility less than the Noack Volatility Factor is isolated. The herein-recited preferred embodiments of the Fischer-Tropsch lubricant base oil also may be isolated from the process. Preferably, the paraffinic wax feed is hydroisomerized using a shape selective intermediate pore size molecular sieve comprising a noble metal hydrogenation component under conditions of about 600° F. to 750° F. Preferred processes for making the Fischer-Tropsch derived lubricant base oils are described in U.S.S.N. 10/744,870, filed Dec. 23, 2003, herein incorporated by reference in its entirety. Examples of embodiments of Fischer-Tropsch lubricant base oil fractions with high monocycloparaffins and low multicycloparaffins are described in U.S.S.N. 10/744,389, filed Dec. 23, 2003, herein incorporated by reference in its entirety.

According to the present invention, the lubricant base oil fractions derived from highly paraffinic wax contain a relatively high weight percent of molecules with cycloparaffinic functionality. In a preferred embodiment, the lubricant base oil fraction derived from highly paraffinic wax comprises greater than 5 weight percent molecules with cycloparaffinic functionality. In another preferred embodiment, the lubricant base oil fraction derived from highly paraffinic wax comprises a ratio of weight percent of molecules with monocycloparaffinic functionality to weight percent of molecules with multicycloparaffinic functionality of greater than 5. The lubricant base oil fraction derived from highly paraffinic wax containing a high ratio of weight percent of molecules with monocycloparaffinic functionality to weight percent of molecules with multicycloparaffinic functionality (or high weight percent of molecules with monocycloparaffinic functionality and low weight percent of molecules with multicycloparaffinic functionality) are exceptional lubricant additive diluent oils and make exceptional oil soluble additive concentrates.

Even though these lubricant base oil fractions derived from highly paraffinic wax contain a high paraffins content, they unexpectedly exhibit solubility for additives, including VI improvers and lubricant additive packages, because cycloparaffins impart additive solubility. These lubricant base oil fractions derived from highly paraffinic wax are also desirable because molecules with multicycloparraffinic functionality reduce oxidation stability, lower viscosity index, and increase Noack volatility. Models of the effects of molecules with multicycloparraffinic functionality are given in V. J. Gatto, et al, "The Influence of Chemical Structure on the Physical Properties and Antioxidant Response of Hydrocracked Base Stocks and Polyalphaolefins," *J. Synthetic Lubrication* 19-1, April 2002, pp 3-18. In addition, the lubricant base oil fractions of the present invention exhibit unexpectedly low volatility and relatively low viscosity.

Accordingly, in a preferred embodiment, the lubricant base oil fractions derived from highly paraffinic wax used as lubricant additive diluent oils in oil soluble additive concentrates comprise very low weight percents of molecules with aromatic functionality, a high weight percent of molecules with cycloparaffinic functionality, and a high ratio of weight percent of molecules with monocycloparraffinic functionality to weight percent of molecules with multicycloparraffinic functionality (or high weight percent of molecules with monocycloparraffinic functionality and very low weight percents of molecules with multicycloparraffinic functionality). The lubricant base oils of the present invention may also have preferred alkyl branching placements.

The lubricant base oil fractions derived from highly paraffinic wax used as lubricant additive diluent oils in oil soluble additive concentrates contain greater than 95 weight % saturates as determined by elution column chromatography, ASTM D 2549-02. Olefins are present in an amount less than detectable by long duration C<sup>13</sup> Nuclear Magnetic Resonance Spectroscopy (NMR). Preferably, molecules with aromatic functionality are present in amounts less than 0.3 weight percent by HPLC-UV, and confirmed by ASTM D 5292-99 modified to measure low level aromatics. In preferred embodiments molecules with aromatic functionality are present in amounts less than 0.10 weight percent, preferably less than 0.05 weight percent, more preferably less than 0.01 weight percent. Sulfur is present in amounts less than 25 ppmw, preferably less than 5 ppmw, and more preferably less than 1 ppmw, as determined by ultraviolet fluorescence by ASTM D 5453-00.

According to the present invention, the lubricant base oil fractions derived from highly paraffinic wax are advantageously used as lubricant additive diluent oils in oil soluble additive concentrates. The oil soluble additive concentrates according to the present invention comprise 5 to 98 weight % of the lubricant base oil fraction derived from highly paraffinic wax and at least 2 weight % of one or more lubricant additives, wherein the lubricant base oil fraction comprises greater than 3 weight % molecules with cycloparraffinic functionality and less than 0.30 weight percent aromatics and has a viscosity of between about 1.0 and 3.5 cSt at 100° C. and a Noack volatility less than the Noack Volatility Factor. The lubricant base oil fraction derived from highly paraffinic wax readily solubilizes the lubricant additives and provides an oil additive concentrate that is readily soluble in the lubricant base oil stocks. In addition, the lubricant base oil fraction derived from highly paraffinic wax does not introduce any undesirable characteristics, including, for example, high volatility, high viscosity, and impurities such as heteroatoms, to the lubricant base oil stocks and thus, ultimately to the finished lubricant. The finished lubricant according to the

present invention comprises the oil soluble additive concentrate and one or more lubricant base oils. The finished lubricant may optionally comprise one or more additional additives and other oil soluble additive concentrates.

5 Definitions and Terms

The following terms will be used throughout the specification and will have the following meanings unless otherwise indicated.

"API CI-4" is a specification of the current engine oil 10 service category of heavy duty engine oils.

"API PC-10" is a specification of the proposed new engine oil service category of heavy duty engine oils. It is expected that PC-10 oils will also have reduced limits for sulfur, in similar amounts as for GF-4 automotive gasoline engine oils.

15 "ILSAC GF-3" is a specification of an engine oil service category of automotive gasoline engines, which became official on Jul. 1, 2001.

"ILSAC GF-4" is a specification of a new engine oil service 20 category of automotive gasoline engines, which was approved on Jan. 8, 2004 and became official on Jul. 1, 2004. This category introduces new sulfur limits by ASTM D 1552. The maximum sulfur limit for 0W and 5W oils is 0.5 weight percent, while the maximum sulfur limit for 10W oils is 0.7 weight percent.

25 "SAE J300 multigrade engine oils" are engine oils defined by the Engine Oil Viscosity Classifications for multigrade engine oils in SAE J300, revised June 2001. The multigrade viscosity types are 0W-XX, 5W-XX, 15W-XX, 20W-XX, and 25W-XX, with XX being 20, 30, 40, 50, or 60. Specific 30 limits are defined for maximum low temperature cranking viscosity by ASTM D 5293, maximum low temperature pumping viscosity with no yield stress by ASTM D 4684, minimum and maximum low shear rate kinematic viscosity at 100° C. by ASTM D 445, and minimum high temperature high shear rate viscosity by ASTM D 4683 or ASTM D 5481.

35 The term "derived from a Fischer-Tropsch process" or "Fischer-Tropsch derived," means that the product, fraction, or feed originates from or is produced at some stage by a Fischer-Tropsch process.

40 The term "derived from a petroleum" or "petroleum derived" means that the product, fraction, or feed originates from the vapor overhead streams from distilling petroleum crude and the residual fuels that are the non-vaporizable remaining portion. A source of the petroleum derived can be 45 from a gas field condensate.

Highly paraffinic wax means a wax having a high content of n-paraffins, generally greater than 40 weight %, preferably greater than 50 weight %, and more preferably greater than 75 weight %. Preferably, the highly paraffinic waxes used in the 50 present invention also have very low levels of nitrogen and sulfur, generally less than 25 ppm total combined nitrogen and sulfur and preferably less than 20 ppm. Examples of highly paraffinic waxes that may be used in the present invention include slack waxes, deoiled slack waxes, refined foots 55 oils, waxy lubricant raffinates, n-paraffin waxes, NAO waxes, waxes produced in chemical plant processes, deoiled petroleum derived waxes, microcrystalline waxes, Fischer-Tropsch waxes, and mixtures thereof. The pour points of the highly paraffinic waxes useful in this invention are greater than 50° C. and preferably greater than 60° C.

60 The term "derived from highly paraffinic wax" means that the product, fraction, or feed originates from or is produced at some stage by from a highly paraffinic wax.

Aromatics means any hydrocarbonaceous compounds that 65 contain at least one group of atoms that share an uninterrupted cloud of delocalized electrons, where the number of delocalized electrons in the group of atom's corresponds to a solution

to the Huckel rule of  $4n+2$  (e.g.,  $n=1$  for 6 electrons, etc.). Representative examples include, but are not limited to, benzene, biphenyl, naphthalene, and the like.

Molecules with cycloparaffinic functionality mean any molecule that is, or contains as one or more substituents, a monocyclic or a fused multicyclic saturated hydrocarbon group. The cycloparaffinic group may be optionally substituted with one or more, preferably one to three, substituents. Representative examples include, but are not limited to, cyclopropyl, cyclobutyl, cyclohexyl, cyclopentyl, cycloheptyl, decahydronaphthalene, octahydronaphthalene, (pentadecan-6-yl)cyclohexane, 3,7,10-tricyclohexylpentadecane, decahydro-1-(pentadecan-6-yl)naphthalene, and the like.

Molecules with monocycloparaffinic functionality mean any molecule that is a monocyclic saturated hydrocarbon group of three to seven ring carbons or any molecule that is substituted with a single monocyclic saturated hydrocarbon group of three to seven ring carbons. The cycloparaffinic group may be optionally substituted with one or more, preferably one to three, substituents. Representative examples include, but are not limited to, cyclopropyl, cyclobutyl, cyclohexyl, cyclopentyl, cycloheptyl, (pentadecan-6-yl)cyclohexane, and the like.

Molecules with multicycloparaffinic functionality mean any molecule that is a fused multicyclic saturated hydrocarbon ring group of two or more fused rings, any molecule that is substituted with one or more fused multicyclic saturated hydrocarbon ring groups of two or more fused rings, or any molecule that is substituted with more than one monocyclic saturated hydrocarbon group of three to seven ring carbons. The fused multicyclic saturated hydrocarbon ring group preferably is of two fused rings. The cycloparaffinic group may be optionally substituted with one or more, preferably one to three, substituents. Representative examples include, but are not limited to, decahydronaphthalene, octahydronaphthalene, 3,7,10-tricyclohexylpentadecane, decahydro-1-(pentadecan-6-yl)naphthalene, and the like.

Brookfield Viscosity: ASTM D 2983-03 is used to determine the low-shear-rate viscosity of automotive fluid lubricants at low temperatures. The low-temperature, low-shear-rate viscosity of automatic transmission fluids, gear oils, torque and tractor fluids, and industrial and automotive hydraulic oils are frequently specified by Brookfield viscosities. The GM 2003 DEXRON® III automatic transmission fluid specification requires a maximum Brookfield viscosity at  $-40^{\circ}\text{C}$ . of 20,000 cP. The Ford MERCON® V specification requires a Brookfield viscosity at  $-40^{\circ}\text{C}$ . between 5,000 and 13,000 cP. The Automotive Gear Lubricant Viscosity Classification SAE J306 for 75W gear lubricants has a low temperature viscosity specification such that the maximum temperature for a viscosity of 150,000 cP is  $-40^{\circ}\text{C}$ . When added to automatic transmission fluid and gear oils, the oil soluble additive concentrates of the present invention do not adversely impact the Brookfield Viscosity at low temperature.

Automotive Gear Lubricant Viscosity Classifications—SAE J306

-continued

| SAE Viscosity Grade | 150,000 cP ( $^{\circ}\text{C}$ .) | Kinematic Viscosity at $100^{\circ}\text{C}$ . (cSt) |      |
|---------------------|------------------------------------|------------------------------------------------------|------|
|                     |                                    | min                                                  | Max  |
| 5                   | 85 W                               | -12                                                  | 11.0 |
|                     | 80                                 | —                                                    | 7.0  |
|                     | 85                                 | —                                                    | 11.0 |
|                     | 90                                 | —                                                    | 13.5 |
|                     | 140                                | —                                                    | 24.0 |
|                     | 250                                | —                                                    | 41.0 |

Kinematic viscosity is a measurement of the resistance to flow of a fluid under gravity. Many lubricant base oils, finished lubricants made from them, and the correct operation of equipment depends upon the appropriate viscosity of the fluid being used. Kinematic viscosity is determined by ASTM D 445-01. The results are reported in centistokes (cSt). The Fischer-Tropsch derived lubricant base oil fractions of the present invention have a kinematic viscosity of between about 1.0 cSt and 3.5 cSt at  $100^{\circ}\text{C}$ . Preferably, the lubricant base oil fractions derived from highly paraffinic wax have a kinematic viscosity of between about 2.0 cSt and 3.5 cSt at  $100^{\circ}\text{C}$ . and more preferably, the lubricant base oil fractions derived from highly paraffinic wax have a kinematic viscosity of between about 2.0 cSt and 3.0 cSt at  $100^{\circ}\text{C}$ .

Viscosity Index (VI) is an empirical, unitless number indicating the effect of temperature change on the kinematic viscosity of the oil. Liquids change viscosity with temperature, becoming less viscous when heated; the higher the VI of an oil, the lower its tendency to change viscosity with temperature. High VI lubricants are needed wherever relatively constant viscosity is required at widely varying temperatures. For example, in an automobile, engine oil must flow freely enough to permit cold starting, but must be viscous enough after warm-up to provide full lubrication. VI may be determined as described in ASTM D 2270-93. Preferably, the lubricant base oil fractions derived from highly paraffinic wax have a viscosity index of between about 105 and 155.

The "Viscosity Index Factor" of the lubricant base oil derived from highly paraffinic wax is an empirical number derived from kinematic viscosity of the lubricant base oil fraction. The viscosity index factor is calculated by the following equation:

$$\text{Viscosity Index Factor} = 28 \times \ln(\text{Kinematic Viscosity of the lubricant base oil fraction at } 100^{\circ}\text{C.}) + 95$$

The lubricant base oil fractions derived from highly paraffinic wax may have a Viscosity Index greater than the Viscosity Index Factor.

Pour point is a measurement of the temperature at which a sample of lubricant base oil will begin to flow under carefully controlled conditions. Pour point may be determined as described in ASTM D 5950-02. The results are reported in degrees Celsius. Many commercial lubricant base oils have specifications for pour point. When lubricant base oils have low pour points, they also are likely to have other good low temperature properties, such as low cloud point, low cold filter plugging point, and low temperature cranking viscosity. Cloud point is a measurement complementary to the pour point, and is expressed as a temperature at which a sample of the lubricant base oil begins to develop a haze under carefully specified conditions. Cloud point may be determined by, for example, ASTM D 5773-95. Lubricant base oils having pour

| SAE Viscosity Grade | 150,000 cP ( $^{\circ}\text{C}$ .) | Kinematic Viscosity at $100^{\circ}\text{C}$ . (cSt) |     |
|---------------------|------------------------------------|------------------------------------------------------|-----|
|                     |                                    | min                                                  | Max |
| 70 W                | -55                                | 4.1                                                  | —   |
| 75 W                | -40                                | 4.1                                                  | —   |
| 80 W                | -26                                | 7.0                                                  | —   |

cloud point spreads below about 35° C. are desirable. Higher pour-cloud point spreads require processing the lubricant base oil to very low pour points in order to meet cloud point specifications.

Noack volatility is defined as the mass of oil, expressed in weight %, which is lost when the oil is heated at 250° C. and 20 mmHg (2.67 kPa; 26.7 mbar) below atmospheric in a test crucible through which a constant flow of air is drawn for 60 minutes, according to ASTM D5800. A more convenient method for calculating Noack volatility and one which correlates well with ASTM D5800 is by using a thermo gravimetric analyzer test (TGA) by ASTM D6375. TGA Noack volatility is used throughout this disclosure unless otherwise stated. Noack volatility of engine oil, as measured by TGA Noack and similar methods, has been found to correlate with oil consumption in passenger car engines. Strict requirements for low volatility are important aspects of several recent engine oil specifications, such as, for example, ACEA A-3 and B-3 in Europe and ILSAC GF-3 in North America. Preferably, the lubricant base oil fractions derived from highly paraffinic wax of the present invention have a Noack volatility of less than 50 weight %. More preferably, the lubricant base oil fractions derived from highly paraffinic wax of the present invention have a Noack volatility of less than 35 weight %.

The "Noack Volatility Factor" of the lubricant base oil derived from highly paraffinic wax is an empirical number derived from kinematic viscosity of the lubricant base oil fraction. The Noack volatility factor is calculated by the following equation:

$$\text{Noack Volatility Factor} = 160 - 40(\text{Kinematic Viscosity at } 100^\circ \text{ C.})$$

The lubricant base oil fractions derived from highly paraffinic wax have a Noack volatility less than the Noack Volatility Factor.

The aniline point test indicates if an oil is likely to damage elastomers (rubber compounds) that come in contact with the oil. The aniline point is called the "aniline point temperature," which is the lowest temperature (° F. or ° C.) at which equal volumes of aniline ( $C_6H_5NH_2$ ) and the oil form a single phase. The aniline point (AP) correlates roughly with the amount and type of aromatic hydrocarbons in an oil sample. A low AP is indicative of higher aromatics, while a high AP is indicative of lower aromatics content. The aniline point is determined by ASTM D611-04. Preferably, the lubricant base oil fractions derived from highly paraffinic wax of the present invention have an aniline point greater than  $36 \times 1n(\text{Kinematic Viscosity of the lubricant base oil fraction at } 100^\circ \text{ C.}) + 200$ . Accordingly, the lubricant base oil fractions derived from highly paraffinic wax exhibit good elastomer compatibility.

The Oxidator BN with L-4 Catalyst Test is a test measuring resistance to oxidation by means of a Dornte-type oxygen absorption apparatus (R. W. Dornte "Oxidation of White Oils," Industrial and Engineering Chemistry, Vol. 28, page 26, 1936). Normally, the conditions are one atmosphere of pure oxygen at 340° F., reporting the hours to absorption of 1000 ml of  $O_2$  by 100 g of oil. In the Oxidator BN with L-4 Catalyst test, 0.8 ml of catalyst is used per 100 grams of oil. The catalyst is a mixture of soluble metal naphthenates in kerosene simulating the average metal analysis of used crankcase oil. The mixture of soluble metal naphthenates simulates the average metal analysis of used crankcase oil. The level of metals in the catalyst is as follows: Copper=6,927 ppm; Iron=4,083 ppm; Lead=80,208 ppm; Manganese=350 ppm; Tin=3565 ppm. The additive package is 80 millimoles of zinc bispolypropylenephenyldithio-phosphate per 100 grams of oil, or approximately 1.1 grams of OLOA® 260. The Oxida-

tor BN with L-4 Catalyst Test measures the response of a finished lubricant in a simulated application. High values, or long times to adsorb one liter of oxygen, indicate good stability. OLOA® is an acronym for Oronite Lubricating Oil Additive®, which is a registered trademark of Chevron-Texaco Oronite Company.

Generally, the Oxidator BN with L-4 Catalyst Test results should be above about 7 hours. Preferably, the Oxidator BN with L-4 value will be greater than about 10 hours. Preferably, the lubricant base oil fraction derived from highly paraffinic wax of the present invention have results greater than about 10 hours. The Fischer-Tropsch derived lubricant base oil fractions of the present invention have results much greater than 10 hours. Preferably, the Fischer-Tropsch derived lubricant base oil fractions of the oil soluble additive concentrates of the present invention have an Oxidator BN with L-4 Catalyst test result of greater than 25 hours.

#### Highly Paraffinic Wax

The highly paraffinic wax used in making the lubricant base oils of the present invention can be any wax having a high content of n-paraffins. Preferably, the highly paraffinic wax comprise greater than 40 weight % n-paraffins, preferably greater than 50 weight %, and more preferably greater than 75 weight %. Preferably, the highly paraffinic waxes used in the present invention also have very low levels of nitrogen and sulfur, generally less than 25 ppm total combined nitrogen and sulfur and preferably less than 20 ppm. Examples of highly paraffinic waxes that may be used in the present invention include slack waxes, deoiled slack waxes, refined foots oils, waxy lubricant raffinates, n-paraffin waxes, NAO waxes, waxes produced in chemical plant processes, deoiled petroleum derived waxes, microcrystalline waxes, Fischer-Tropsch waxes, and mixtures thereof. The pour points of the highly paraffinic waxes useful in this invention are greater than 50° C. and preferably greater than 60° C.

It has been discovered that these highly paraffinic waxes can be processed to provide lubricant base oil fractions having low volatility and low viscosity and unexpectedly also having good additive solubility. In one preferred embodiment, the highly paraffinic wax is a Fischer-Tropsch derived wax and provides a Fischer-Tropsch derived lubricant base oil fraction.

#### Fischer-Tropsch Synthesis

In Fischer-Tropsch chemistry, syngas is converted to liquid hydrocarbons by contact with a Fischer-Tropsch catalyst under reactive conditions. Typically, methane and optionally heavier hydrocarbons (ethane and heavier) can be sent through a conventional syngas generator to provide synthesis gas. Generally, synthesis gas contains hydrogen and carbon monoxide, and may include minor amounts of carbon dioxide and/or water. The presence of sulfur, nitrogen, halogen, selenium, phosphorus and arsenic contaminants in the syngas is undesirable. For this reason and depending on the quality of the syngas, it is preferred to remove sulfur and other contaminants from the feed before performing the Fischer-Tropsch chemistry. Means for removing these contaminants are well known to those of skill in the art. For example, ZnO guard-beds are preferred for removing sulfur impurities. Means for removing other contaminants are well known to those of skill in the art. It also may be desirable to purify the syngas prior to the Fischer-Tropsch reactor to remove carbon dioxide produced during the syngas reaction and any additional sulfur compounds not already removed. This can be accomplished, for example, by contacting the syngas with a mildly alkaline solution (e.g., aqueous potassium carbonate) in a packed column.

## 11

In the Fischer-Tropsch process, contacting a synthesis gas comprising a mixture of H<sub>2</sub> and CO with a Fischer-Tropsch catalyst under suitable temperature and pressure reactive conditions forms liquid and gaseous hydrocarbons. The Fischer-Tropsch reaction is typically conducted at temperatures of about 300-700° F. (149-371° C.), preferably about 400-550° F. (204-228° C.); pressures of about 10-600 psia, (0.7-41 bars), preferably about 30-300 psia, (2-21 bars); and catalyst space velocities of about 100-10,000 cc/g/hr, preferably about 300-3,000 cc/g/hr. Examples of conditions for performing Fischer-Tropsch type reactions are well known to those of skill in the art.

The products of the Fischer-Tropsch synthesis process may range from C<sub>1</sub> to C<sub>200+</sub> with a majority in the C<sub>5</sub> to C<sub>100+</sub> range. The reaction can be conducted in a variety of reactor types, such as fixed bed reactors containing one or more catalyst beds, slurry reactors, fluidized bed reactors, or a combination of different type reactors. Such reaction processes and reactors are well known and documented in the literature.

The slurry Fischer-Tropsch process, which is preferred in the practice of the invention, utilizes superior heat (and mass) transfer characteristics for the strongly exothermic synthesis reaction and is able to produce relatively high molecular weight, paraffinic hydrocarbons when using a cobalt catalyst. In the slurry process, a syngas comprising a mixture of hydrogen and carbon monoxide is bubbled up as a third phase through a slurry which comprises a particulate Fischer-Tropsch type hydrocarbon synthesis catalyst dispersed and suspended in a slurry liquid comprising hydrocarbon products of the synthesis reaction which are liquid under the reaction conditions. The mole ratio of the hydrogen to the carbon monoxide may broadly range from about 0.5 to about 4, but is more typically within the range of from about 0.7 to about 2.75 and preferably from about 0.7 to about 2.5. A particularly preferred Fischer-Tropsch process is taught in EP0609079, also completely incorporated herein by reference for all purposes.

In general, Fischer-Tropsch catalysts contain a Group VIII transition metal on a metal oxide support. The catalysts may also contain a noble metal promoter(s) and/or crystalline molecular sieves. Suitable Fischer-Tropsch catalysts comprise one or more of Fe, Ni, Co, Ru and Re, with cobalt being preferred. A preferred Fischer-Tropsch catalyst comprises effective amounts of cobalt and one or more of Re, Ru, Pt, Fe, Ni, Th, Zr, Hf, U, Mg and La on a suitable inorganic support material, preferably one which comprises one or more refractory metal oxides. In general, the amount of cobalt present in the catalyst is between about 1 and about 50 weight percent of the total catalyst composition. The catalysts can also contain basic oxide promoters such as ThO<sub>2</sub>, La<sub>2</sub>O<sub>3</sub>, MgO, and TiO<sub>2</sub>, promoters such as ZrO<sub>2</sub>, noble metals (Pt, Pd, Ru, Rh, Os, Ir), coinage metals (Cu, Ag, Au), and other transition metals such as Fe, Mn, Ni, and Re. Suitable support materials include alumina, silica, magnesia and titania or mixtures thereof. Preferred supports for cobalt containing catalysts comprise titania. Useful catalysts and their preparation are known and illustrated in U.S. Pat. No. 4,568,663, which is intended to be illustrative but non-limiting relative to catalyst selection.

Certain catalysts are known to provide chain growth probabilities that are relatively low to moderate, and the reaction products include a relatively high proportion of low molecular (C<sub>2-8</sub>) weight olefins and a relatively low proportion of high molecular weight (C<sub>30+</sub>) waxes. Certain other catalysts are known to provide relatively high chain growth probabilities, and the reaction products include a relatively low proportion of low molecular (C<sub>2-8</sub>) weight olefins and a rela-

## 12

tively high proportion of high molecular weight (C<sub>30+</sub>) waxes. Such catalysts are well known to those of skill in the art and can be readily obtained and/or prepared.

The product from a Fischer-Tropsch process contains predominantly paraffins. The products from Fischer-Tropsch reactions generally include a light reaction product and a waxy reaction product. The light reaction product (i.e., the condensate fraction) includes hydrocarbons boiling below about 700° F. (e.g., tail gases through middle distillate fuels), largely in the C<sub>5</sub>-C<sub>20</sub> range, with decreasing amounts up to about C<sub>30</sub>. The waxy reaction product (i.e., the wax fraction) includes hydrocarbons boiling above about 600° F. (e.g., vacuum gas oil through heavy paraffins), largely in the C<sub>20+</sub> range, with decreasing amounts down to C<sub>10</sub>.

Both the light reaction product and the waxy product are substantially paraffinic. The waxy product generally comprises greater than 70 weight % normal paraffins, and often greater than 80 weight % normal paraffins. The light reaction product comprises paraffinic products with a significant proportion of alcohols and olefins. In some cases, the light reaction product may comprise as much as 50 weight %, and even higher, alcohols and olefins. It is the waxy reaction product (i.e., the wax fraction) that is used as a feedstock to the process for providing the Fischer-Tropsch derived lubricant base oil fraction used as a lubricant additive diluent oil in the oil soluble concentrates and finished lubricants according to the present invention.

The Fischer-Tropsch lubricant base oil fractions used as lubricant additive diluent oils in the oil soluble additive concentrates are prepared from the waxy fractions of the Fischer-Tropsch syncrude by a process including hydroisomerization. Preferably, the Fischer-Tropsch lubricant base oils are made by a process as described in U.S.S.N. 10/744,870, filed Dec. 23, 2003, herein incorporated by reference in its entirety. The Fischer-Tropsch lubricant base oil fractions used in the oil soluble additive concentrates according to the present invention may be manufactured at a site different from the site at which the components of the oil soluble additive concentrates are received and blended and at a site different from the site at which the oil soluble additive concentrate is blended with lubricant base oil stocks to provide a finished lubricant. The site at which the oil soluble additive concentrate is made may be the same or different than the site at which the finished lubricant is made.

## 45 Process for Providing Light Lubricant Base Oil Fraction

These light lubricant base oil fractions derived from highly paraffinic wax of the present invention are made by process comprising providing a highly paraffinic wax and then hydroisomerizing the highly paraffinic wax to provide the lubricant base oil fractions as described herein. Preferably, the highly paraffinic wax is hydroisomerized using a shape selective intermediate pore size molecular sieve comprising a noble metal hydrogenation component under conditions of about 600° F. to 750° F.

55 In one preferred embodiment, the highly paraffinic wax is a Fischer-Tropsch derived wax and provides a Fischer-Tropsch derived lubricant base oil fraction. The Fischer-Tropsch derived lubricant base oil fraction used in the oil soluble additive concentrate is made by a Fischer-Tropsch synthesis process followed by hydroisomerization of the waxy fractions of the Fischer-Tropsch syncrude.

## Hydroisomerization

The highly paraffinic waxes are subjected to a process comprising hydroisomerization to provide the lubricant base oil fractions useful as lubricant additive diluent oils in oil soluble additive concentrates according to the present invention.

Hydroisomerization is intended to improve the cold flow properties of the lubricant base oil by the selective addition of branching into the molecular structure. Hydroisomerization ideally will achieve high conversion levels of the highly paraffinic wax to non-waxy iso-paraffins while at the same time minimizing the conversion by cracking. Preferably, the conditions for hydroisomerization in the present invention are controlled such that the conversion of the compounds boiling above about 700° F. in the wax feed to compounds boiling below about 700° F. is maintained between about 10 wt % and 50 wt%, preferably between 15 wt% and 45 wt%.

According to the present invention, hydroisomerization is conducted using a shape selective intermediate pore size molecular sieve. Hydroisomerization catalysts useful in the present invention comprise a shape selective intermediate pore size molecular sieve and optionally a catalytically active metal hydrogenation component on a refractory oxide support. The phrase "intermediate pore size," as used herein means an effective pore aperture in the range of from about 3.9 to about 7.1 Å when the porous inorganic oxide is in the calcined form. The shape selective intermediate pore size molecular sieves used in the practice of the present invention are generally 1-D 10-, 11- or 12-ring molecular sieves. The preferred molecular sieves of the invention are of the 1-D 10-ring variety, where 10-(or 11- or 12-) ring molecular sieves have 10 (or 11 or 12) tetrahedrally-coordinated atoms (T-atoms) joined by oxygens. In the 1-D molecular sieve, the 10-ring (or larger) pores are parallel with each other, and do not interconnect. Note, however, that 1-D 10-ring molecular sieves which meet the broader definition of the intermediate pore size molecular sieve but include intersecting pores having 8-membered rings may also be encompassed within the definition of the molecular sieve of the present invention. The classification of intrazeolite channels as 1-D, 2-D and 3-D is set forth by R. M. Barrer in *Zeolites, Science and Technology*, edited by F. R. Rodrigues, L. D. Rollman and C. Naccache, NATO ASI Series, 1984 which classification is incorporated in its entirety by reference (see particularly page 75).

Preferred shape selective intermediate pore size molecular sieves used for hydroisomerization are based upon aluminum phosphates, such as SAPO-11, SAPO-31, and SAPO-41. SAPO-11 and SAPO-31 are more preferred, with SAPO-11 being most preferred. SM-3 is a particularly preferred shape selective intermediate pore size SAPO, which has a crystalline structure falling within that of the SAPO-11 molecular sieves. The preparation of SM-3 and its unique characteristics are described in U.S. Pat. Nos. 4,943,424 and 5,158,665. Also preferred shape selective intermediate pore size molecular sieves used for hydroisomerization are zeolites, such as ZSM-22, ZSM-23, ZSM-35, ZSM-48, ZSM-57, SSZ-32, offretite, and ferrierite. SSZ-32 and ZSM-23 are more preferred.

A preferred intermediate pore size molecular sieve is characterized by selected crystallographic free diameters of the channels, selected crystallite size (corresponding to selected channel length), and selected acidity. Desirable crystallographic free diameters of the channels of the molecular sieves are in the range of from about 3.9 to about 7.1 Angstrom, having a maximum crystallographic free diameter of not more than 7.1 and a minimum crystallographic free diameter of not less than 3.9 Angstrom. Preferably the maximum crystallographic free diameter is not more than 7.1 and the minimum crystallographic free diameter is not less than 4.0 Angstrom. Most preferably the maximum crystallographic free diameter is not more than 6.5 and the minimum crystallographic free diameter is not less than 4.0 Angstrom. The crystallographic free diameters of the channels of molecular sieves are published in the "Atlas of Zeolite Framework

Types", Fifth Revised Edition, 2001, by Ch. Baerlocher, W. M. Meier, and D. H. Olson, Elsevier, pp 10-15, which is incorporated herein by reference.

A particularly preferred intermediate pore size molecular sieve, which is useful in the present process is described, for example, in U.S. Pat. Nos. 5,135,638 and 5,282,958, the contents of which are hereby incorporated by reference in their entirety. In U.S. Pat. No. 5,282,958, such an intermediate pore size molecular sieve has a crystallite size of no more than about 0.5 microns and pores with a minimum diameter of at least about 4.8 Å and with a maximum diameter of about 7.1 Å. The catalyst has sufficient acidity so that 0.5 grams thereof when positioned in a tube reactor converts at least 50% of hexadecane at 370° C., a pressure of 1200 psig, a hydrogen flow of 160 ml/min, and a feed rate of 1 ml/hr. The catalyst also exhibits isomerization selectivity of 40 percent or greater (isomerization selectivity is determined as follows:  $100 \times (\text{weight \% branched C}_{16} \text{ in product}) / (\text{weight \% branched C}_{16} \text{ in product} + \text{weight \% C}_{13-} \text{ in product})$  when used under conditions leading to 96% conversion of normal hexadecane (n-C<sub>16</sub>) to other species.

Such a particularly preferred molecular sieve may further be characterized by pores or channels having a crystallographic free diameter in the range of from about 4.0 to about 7.1 Å, and preferably in the range of 4.0 to 6.5 Å. The crystallographic free diameters of the channels of molecular sieves are published in the "Atlas of Zeolite Framework Types", Fifth Revised Edition, 2001, by Ch. Baerlocher, W. M. Meier, and D. H. Olson, Elsevier, pp 10-15, which is incorporated herein by reference.

If the crystallographic free diameters of the channels of a molecular sieve are unknown, the effective pore size of the molecular sieve can be measured using standard adsorption techniques and hydrocarbonaceous compounds of known minimum kinetic diameters. See Breck, *Zeolite Molecular Sieves*, 1974 (especially Chapter 8); Anderson et al. *J. Catalysis* 58, 114 (1979); and U.S. Pat. No. 4,440,871, the pertinent portions of which are incorporated herein by reference. In performing adsorption measurements to determine pore size, standard techniques are used. It is convenient to consider a particular molecule as excluded if does not reach at least 95% of its equilibrium adsorption value on the molecular sieve in less than about 10 minutes ( $p/p_\infty = 0.5$  at 25° C.). Intermediate pore size molecular sieves will typically admit molecules having kinetic diameters of 5.3 to 6.5 Angstrom with little hindrance.

Hydroisomerization catalysts useful in the present invention comprise a catalytically active hydrogenation metal. The presence of a catalytically active hydrogenation metal leads to product improvement, especially VI and stability. Typical catalytically active hydrogenation metals include chromium, molybdenum, nickel, vanadium, cobalt, tungsten, zinc, platinum, and palladium. The metals platinum and palladium are especially preferred, with platinum most especially preferred. If platinum and/or palladium is used, the total amount of active hydrogenation metal is typically in the range of 0.1 to 5 weight percent of the total catalyst, usually from 0.1 to 2 weight percent, and not to exceed 10 weight percent.

The refractory oxide support may be selected from those oxide supports, which are conventionally used for catalysts, including silica, alumina, silica-alumina, magnesia, titania and combinations thereof.

The conditions for hydroisomerization will be tailored to achieve a lubricant base oil fraction comprising less than about 0.3 weight % aromatics and greater than 3 weight % molecules with cycloparaffinic functionality. Preferably, the conditions provide a lubricant base oil fraction comprising

## 15

greater than 5 weight % molecules with cycloparaffinic functionality and a ratio of weight percent of molecules with monocycloparaffinic functionality of weight percent of molecules with multicycloparaffinic functionality of greater than 5, more preferably greater than 15, and even more preferably greater than 50. The conditions for hydroisomerization will depend on the properties of feed used, the catalyst used, whether or not the catalyst is sulfided, the desired yield, and the desired properties of the lubricant base oil. Conditions under which the hydroisomerization process of the current invention may be carried out include temperatures from about 500° F. to about 775° F. (260° C. to about 413° C.), preferably 600° F. to about 750° F. (315° C. to about 399° C.), more preferably about 600° F. to about 700° F. (315° C. to about 371° C.); and pressures from about 15 to 3000 psig, preferably 100 to 2500 psig. The hydroisomerization pressures in this context refer to the hydrogen partial pressure within the hydroisomerization reactor, although the hydrogen partial pressure is substantially the same (or nearly the same) as the total pressure. The liquid hourly space velocity during contacting is generally from about 0.1 to 20 hr<sup>-1</sup>, preferably from about 0.1 to about 5 hr<sup>-1</sup>. The hydrogen to hydrocarbon ratio falls within a range from about 1.0 to about 50 moles H<sub>2</sub> per mole hydrocarbon, more preferably from about 10 to about 20 moles H<sub>2</sub> per mole hydrocarbon. Suitable conditions for performing hydroisomerization are described in U.S. Pat. Nos. 5,282,958 and 5,135,638, the contents of which are incorporated by reference in their entirety.

Hydrogen is present in the reaction zone during the hydroisomerization process, typically in a hydrogen to feed ratio from about 0.5 to 30 MSCF/bbl (thousand standard cubic feet per barrel), preferably from about 1 to about 10 MSCF/bbl. Hydrogen may be separated from the product and recycled to the reaction zone.

## Hydrotreating

The highly paraffinic waxy feed to the hydroisomerization process may be hydrotreated prior to hydroisomerization. Hydrotreating refers to a catalytic process, usually carried out in the presence of free hydrogen, in which the primary purpose is the removal of various metal contaminants, such as arsenic, aluminum, and cobalt; heteroatoms, such as sulfur and nitrogen; oxygenates; or aromatics from the feed stock. Generally, in hydrotreating operations cracking of the hydrocarbon molecules, i.e., breaking the larger hydrocarbon molecules into smaller hydrocarbon molecules, is minimized, and the unsaturated hydrocarbons are either fully or partially hydrogenated.

Catalysts used in carrying out hydrotreating operations are well known in the art. See, for example, U.S. Pat. Nos. 4,347,121 and 4,810,357, the contents of which are hereby incorporated by reference in their entirety, for general descriptions of hydrotreating, hydrocracking, and of typical catalysts used in each of the processes. Suitable catalysts include noble metals from Group VIII A (according to the 1975 rules of the International Union of Pure and Applied Chemistry), such as platinum or palladium on an alumina or siliceous matrix, and Group VIII and Group VIB, such as nickel-molybdenum or nickel-tin on an alumina or siliceous matrix. U.S. Pat. No. 3,852,207 describes a suitable noble metal catalyst and mild conditions. Other suitable catalysts are described, for example, in U.S. Pat. Nos. 4,157,294 and 3,904,513. The non-noble hydrogenation metals, such as nickel-molybdenum, are usually present in the final catalyst composition as oxides, but are usually employed in their reduced or sulfided forms when such sulfide compounds are readily formed from the particular metal involved. Preferred non-noble metal catalyst compositions contain in excess of about 5 weight percent,

## 16

preferably about 5 to about 40 weight percent molybdenum and/or tungsten, and at least about 0.5, and generally about 1 to about 15 weight percent of nickel and/or cobalt determined as the corresponding oxides. Catalysts containing noble metals, such as platinum, contain in excess of 0.01 percent metal, preferably between 0.1 and 1.0 percent metal. Combinations of noble metals may also be used, such as mixtures of platinum and palladium.

Typical hydrotreating conditions vary over a wide range. In general, the overall LHSV is about 0.25 to 2.0, preferably about 0.5 to 1.5. The hydrogen partial pressure is greater than 200 psia, preferably ranging from about 500 psia to about 2000 psia. Hydrogen recirculation rates are typically greater than 50 SCF/Bbl, and are preferably between 1000 and 5000 SCF/Bbl. Temperatures in the reactor will range from about 300° F. to about 750° F. (about 150° C. to about 400° C.), preferably ranging from 450° F. to 725° F. (230° C. to 385° C.).

## Hydrofinishing

Hydrofinishing is a hydrotreating process that may be used as a step following hydroisomerization to provide the lubricant base oil fractions derived from highly paraffinic wax. Hydrofinishing is intended to improve oxidation stability, UV stability, and appearance of the lubricant base oil fractions by removing traces of aromatics, olefins, color bodies, and solvents. As used in this disclosure, the term UV stability refers to the stability of the lubricant base oil fraction or the finished lubricant when exposed to UV light and oxygen. Instability is indicated when a visible precipitate forms, usually seen as floc or cloudiness, or a darker color develops upon exposure to ultraviolet light and air. A general description of hydrofinishing may be found in U.S. Pat. Nos. 3,852,207 and 4,673,487.

The lubricant base oil fractions derived from highly paraffinic wax of the present invention may be hydrofinished to improve product quality and stability. During hydrofinishing, overall liquid hourly space velocity (LHSV) is about 0.25 to 2.0 hr<sub>-1</sub>, preferably about 0.5 to 1.0 hr<sub>-1</sub>. The hydrogen partial pressure is greater than 200 psia, preferably ranging from about 500 psia to about 2000 psia. Hydrogen recirculation rates are typically greater than 50 SCF/Bbl, and are preferably between 1000 and 5000 SCF/Bbl. Temperatures range from about 300° F. to about 750° F., preferably ranging from 450° F. to 600° F.

Suitable hydrofinishing catalysts include noble metals from Group VIII A (according to the 1975 rules of the International Union of Pure and Applied Chemistry), such as platinum or palladium on an alumina or siliceous matrix, and unsulfided Group VIII A and Group VIB, such as nickel-molybdenum or nickel-tin on an alumina or siliceous matrix. U.S. Pat. No. 3,852,207 describes a suitable noble metal catalyst and mild conditions. Other suitable catalysts are described, for example, in U.S. Pat. Nos. 4,157,294 and 3,904,513. The non-noble metal (such as nickel-molybdenum and/or tungsten, and at least about 0.5, and generally about 1 to about 15 weight percent of nickel and/or cobalt determined as the corresponding oxides. The noble metal (such as platinum) catalyst contains in excess of 0.01 percent metal, preferably between 0.1 and 1.0 percent metal. Combinations of noble metals may also be used, such as mixtures of platinum and palladium.

Clay treating to remove impurities is an alternative final process step to provide lubricant base oil fractions derived from highly paraffinic wax.

## Fractionation

Optionally, the process to provide the light lubricant base oil fractions derived from highly paraffinic wax may include

fractionating the highly paraffinic wax feed prior to hydroisomerization, or fractionating of the lubricant base oil obtained from the hydroisomerization process. The fractionation of the highly paraffinic wax feed or the isomerized lubricant base oil into fractions is generally accomplished by either atmospheric or vacuum distillation, or by a combination of atmospheric and vacuum distillation. Atmospheric distillation is typically used to separate the lighter distillate fractions, such as naphtha and middle distillates, from a bottoms fraction having an initial boiling point above about 600° F. to about 750° F. (about 315° C. to about 399° C.). At higher temperatures thermal cracking of the hydrocarbons may take place leading to fouling of the equipment and to lower yields of the heavier cuts. Vacuum distillation is typically used to separate the higher boiling material, such as the lubricant base oil fractions, into different boiling range cuts. Fractionating the lubricant base oil into different boiling range cuts enables the lubricant base oil manufacturing plant to produce more than one grade, or viscosity, of lubricant base oil.

#### Solvent Dewaxing

The process to make the lubricant base oil fractions derived from highly paraffinic wax may also include a solvent dewaxing step following the hydroisomerization process. Solvent dewaxing optionally may be used to remove small amounts of remaining waxy molecules from the lubricant base oil after hydroisomerization. Solvent dewaxing is done by dissolving the lubricant base oil in a solvent, such as methyl ethyl ketone, methyl iso-butyl ketone, or toluene, or precipitating the wax molecules as discussed in *Chemical Technology of Petroleum*, 3rd Edition, William Gruse and Donald Stevens, McGraw-Hill Book Company, Inc., New York, 1960, pages 566 to 570. Solvent dewaxing is also described in U.S. Pat. Nos. 4,477,333, 3,773,650 and 3,775,288.

#### Lubricant Base Oil Fraction Derived from Highly Paraffinic Wax

The light lubricant base oil fraction derived from highly paraffinic wax according to the present invention is suitable for use as a lubricant additive diluent oil in oil soluble additive concentrates. The lubricant base oil fraction derived from highly paraffinic wax has a viscosity of between about 1.0 cSt and 3.5 cSt at 100° C., preferably between about 2 cSt and 3.5 cSt at 100° C., and more preferably between about 2 cSt and 3.0 cSt at 100° C. Given the relatively low kinematic viscosity, the lubricant base oil fraction derived from highly paraffinic wax advantageously has a high Noack volatility. The lubricant base oil fraction derived from highly paraffinic wax has a Noack volatility less than the Noack volatility factor as calculated by the following equation:

$$\text{Noack Volatility Factor} = 160 - 40(\text{Kinematic Viscosity at } 100^\circ \text{ C.})$$

Preferably, the lubricant base oil fraction derived from highly paraffinic wax has a Noack volatility of less than 50 weight % and preferably, less than 35 weight %. Accordingly, the lubricant base oil fractions derived from highly paraffinic wax of the present invention advantageously have both low viscosity and low volatility.

In certain preferred embodiments, the lubricant base oil fractions derived from highly paraffinic wax has a VI of between about 105 and 155.

Preferably, the Viscosity Index of the lubricant base oil fraction derived from highly paraffinic wax is greater than the Viscosity Index Factor as calculated by the following equation:

$$\text{Viscosity Index Factor} = 28 \times \ln(\text{Kinematic Viscosity of the Fischer-Tropsch derived base oil fraction at } 100^\circ \text{ C.}) + 95.$$

In other preferred embodiments, the lubricant base oil fractions derived from highly paraffinic wax comprise a weight % of molecules with cycloparaffinic functionality of greater than the kinematic viscosity at 100° C. multiplied by three.

5 The lubricant base oil fractions according to the present invention have good low volatilities so that they do not contribute volatility to the finished lubricant, while also being not so heavy as to thicken the finished lubricant. Accordingly, these lubricant base oil fractions have low volatility and low viscosity.

10 The lubricant base oil fractions according to the present invention comprise extremely low levels of unsaturates. The lubricant base oil fraction comprises less than 0.30 weight percent aromatics and greater than 3 weight % molecules with cycloparaffinic functionality. Preferably, the lubricant base oil fraction comprises a ratio of weight percent of molecules with monocycloparaffinic functionality to weight percent of molecules with multicycloparaffinic functionality of greater than 5.

15 20 In a preferred embodiment, the lubricant base oil fraction comprises greater than 5 weight percent molecules with cycloparaffinic functionality. In other preferred embodiments, the lubricant base oil fraction used in the oil soluble additive concentrates comprises a ratio of weight % of molecules with monocycloparaffinic functionality to weight % of molecules with multicycloparaffinic functionality of greater than 5, preferably greater than 15, and more preferably greater than 50. In another preferred embodiment, the lubricant base oil fraction comprises a ratio of weight percent of molecules with cycloparaffinic functionality of greater than the kinematic viscosity at 100° C. multiplied by three.

25 30 In preferred embodiments, the lubricant base oil fraction comprises greater than 9 alkyl branches/100 carbons. The lubricant base oil fraction used as lubricant additive diluent oils in the oil soluble additive concentrates may also have preferred alkyl branching placements. As such, the lubricant base oils of the present invention may comprise predominantly methyl branching. The branching may be such that there are 6 to 18 alkyl branches per 100 carbon; greater than 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660

by long duration C<sup>13</sup> Nuclear Magnetic Resonance Spectroscopy (NMR). Preferably, molecules with aromatic functionality are present in amounts less than 0.3 weight percent by HPLC-UV, and confirmed by ASTM D 5292-99 modified to measure low level aromatics. In preferred embodiments molecules with at least aromatic functionality are present in amounts less than 0.10 weight percent, preferably less than 0.05 weight percent, more preferably less than 0.01 weight percent. Sulfur is present in amounts less than 25 ppm, preferably less than 5 ppm, and more preferably less than 1 ppm as determined by ultraviolet fluorescence by ASTM D 5453-00.

The lubricant base oil fraction derived from highly paraffinic wax readily solubilizes lubricant additives and provides an oil additive concentrate that is readily soluble in the lubricant base oil stocks. In addition, the lubricant base oil fraction do not introduce any undesirable characteristics, including, for example, high volatility, high viscosity, and impurities such as heteroatoms, to the lubricant base oil stocks and thus, ultimately to the finished lubricant.

In a preferred embodiment, the lubricant base oil fraction according to the present invention is a Fischer-Tropsch derived lubricant base oil fraction. Fischer-Tropsch derived waxes are particularly well suited for providing Fischer-Tropsch derived lubricant base oil fractions with the above-described properties.

#### Aromatics Measurement by HPLC-UV:

The method used to measure low levels of molecules with aromatic functionality in the lubricant base oils uses a Hewlett Packard 1050 Series Quaternary Gradient High Performance Liquid Chromatography (HPLC) system coupled with a HP 1050 Diode-Array UV-Vis detector interfaced to an HP Chem-station. Identification of the individual aromatic classes in the highly saturated lubricant base oils was made on the basis of their UV spectral pattern and their elution time. The amino column used for this analysis differentiates aromatic molecules largely on the basis of their ring-number (or more correctly, double-bond number). Thus, the single ring aromatic containing molecules would elute first, followed by the polycyclic aromatics in order of increasing double bond number per molecule. For aromatics with similar double bond character, those with only alkyl substitution on the ring would elute sooner than those with cycloparaffinic substitution.

Unequivocal identification of the various base oil aromatic hydrocarbons from their UV absorbance spectra was somewhat complicated by the fact their peak electronic transitions were all red-shifted relative to the pure model compound analogs to a degree dependent on the amount of alkyl and cycloparaffinic substitution on the ring system. These bathochromic shifts are well known to be caused by alkyl-group delocalization of the  $\pi$ -electrons in the aromatic ring. Since few unsubstituted aromatic compounds boil in the lubricant range, some degree of red-shift was expected and observed for all of the principle aromatic groups identified.

Quantification of the eluting aromatic compounds was made by integrating chromatograms made from wavelengths optimized for each general class of compounds over the appropriate retention time window for that aromatic. Retention time window limits for each aromatic class were determined by manually evaluating the individual absorbance spectra of eluting compounds at different times and assigning them to the appropriate aromatic class based on their qualitative similarity to model compound absorption spectra. With few exceptions, only five classes of aromatic compounds were observed in highly saturated API Group II and III lubricant base oils.

#### HPLC-UV Calibration:

HPLC-UV is used for identifying these classes of aromatic compounds even at very low levels. Multi-ring aromatics typically absorb 10 to 200 times more strongly than single-ring aromatics. Alkyl-substitution also affected absorption by about 20%. Therefore, it is important to use HPLC to separate and identify the various species of aromatics and know how efficiently they absorb.

Five classes of aromatic compounds were identified. With the exception of a small overlap between the most highly retained alkyl-cycloalkyl-1-ring aromatics and the least highly retained alkyl naphthalenes, all of the aromatic compound classes were baseline resolved. Integration limits for the co-eluting 1-ring and 2-ring aromatics at 272nm were made by the perpendicular drop method. Wavelength dependent response factors for each general aromatic class were first determined by constructing Beer's Law plots from pure model compound mixtures based on the nearest spectral peak absorbances to the substituted aromatic analogs.

For example, alkyl-cyclohexylbenzene molecules in base oils exhibit a distinct peak absorbance at 272nm that corresponds to the same (forbidden) transition that unsubstituted tetralin model compounds do at 268nm. The concentration of alkyl-cycloalkyl-1-ring aromatics in base oil samples was calculated by assuming that its molar absorptivity response factor at 272nm was approximately equal to tetralin's molar absorptivity at 268nm, calculated from Beer's law plots. Weight percent concentrations of aromatics were calculated by assuming that the average molecular weight for each aromatic class was approximately equal to the average molecular weight for the whole base oil sample.

This calibration method was further improved by isolating the 1-ring aromatics directly from the lubricant base oils via exhaustive HPLC chromatography. Calibrating directly with these aromatics eliminated the assumptions and uncertainties associated with the model compounds. As expected, the isolated aromatic sample had a lower response factor than the model compound because it was more highly substituted.

More specifically, to accurately calibrate the HPLC-UV method, the substituted benzene aromatics were separated from the bulk of the lubricant base oil using a Waters semi-preparative HPLC unit. 10 grams of sample was diluted 1:1 in n-hexane and injected onto an amino-bonded silica column, a 5cm $\times$ 22.4 mm ID guard, followed by two 25cm $\times$ 22.4 mm ID columns of 8-12 micron amino-bonded silica particles, manufactured by Rainin Instruments, Emeryville, Calif., with n-hexane as the mobile phase at a flow rate of 18 mls/min. Column eluent was fractionated based on the detector response from a dual wavelength UV detector set at 265 nm and 295 nm. Saturate fractions were collected until the 265 nm absorbance showed a change of 0.01 absorbance units, which signaled the onset of single ring aromatic elution. A single ring aromatic fraction was collected until the absorbance ratio between 265 nm and 295 nm decreased to 2.0, indicating the onset of two ring aromatic elution. Purification and separation of the single ring aromatic fraction was made by re-chromatographing the monoaromatic fraction away from the "tailing" saturates fraction which resulted from overloading the HPLC column.

This purified aromatic "standard" showed that alkyl substitution decreased the molar absorptivity response factor by about 20% relative to unsubstituted tetralin.

#### Confirmation of Aromatics by NMR:

The weight percent of molecules with aromatic functionality in the purified mono-aromatic standard was confirmed via long-duration carbon 13 NMR analysis. NMR was easier to calibrate than HPLC UV because it simply measured aro-

matic carbon so the response did not depend on the class of aromatics being analyzed. The NMR results were translated from % aromatic carbon to % aromatic molecules (to be consistent with HPLC-UV and D 2007) by knowing that 95-99% of the aromatics in highly saturated lubricant base oils were single-ring aromatics.

High power, long duration, and good baseline analysis were needed to accurately measure aromatics down to 0.2% aromatic molecules.

More specifically, to accurately measure low levels of all molecules with at least one aromatic function by NMR, the standard D 5292-99 method was modified to give a minimum carbon sensitivity of 500:1 (by ASTM standard practice E 386). A 15-hour duration run on a 400-500 MHz NMR with a 10-12 mm Nalorac probe was used. Acorn PC integration software was used to define the shape of the baseline and consistently integrate. The carrier frequency was changed once during the run to avoid artifacts from imaging the aliphatic peak into the aromatic region. By taking spectra on either side of the carrier spectra, the resolution was improved significantly.

#### Cycloparaffin Distribution by FIMS:

Paraffins are considered more stable than cycloparaffins towards oxidation, and therefore, more desirable. Monocycloparaffins are considered more stable than multicycloparaffins towards oxidation. However, when the weight percent of all molecules with at least one cycloparaffinic function is very low in an oil, the additive solubility is low and the elastomer compatibility is poor. Examples of oils with these properties are Fischer-Tropsch oils (GTL oils) with less than about 5% cycloparaffins. To improve these properties in finished products, expensive co-solvents such as esters must often be added. Preferably, the oil fractions, derived from highly paraffinic wax and used as dielectric fluids, comprise a high weight percent of molecules with monocycloparaffinic functionality and a low weight percent of molecules with multicycloparaffinic functionality such that the oil fractions have high oxidation stability, low volatility, good miscibility with other oils, good additive solubility, and good elastomer compatibility.

The lubricant base oils of this invention were characterized by FIMS into alkanes and molecules with different numbers of unsaturations. The distribution of molecules in the oil fractions was determined by field ionization mass spectroscopy (FIMS). FIMS spectra were obtained on a Micromass VG 70VSE mass spectrometer. The samples were introduced via a solid probe into the spectrophotometer, preferably by placing a small amount (about 0.1 mg) of the base oil to be tested in a glass capillary tube. The capillary tube was placed at the tip of a solids probe for a mass spectrometer, and the probe was heated from about 40° C. up to 500° C. at a rate of 50° C. per minute, operating under vacuum at approximately 10<sup>-6</sup> Torr. The mass spectrometer was scanned from m/z 40 to m/z 1000 at a rate of 5 seconds per decade. The acquired mass spectra were summed to generate one “averaged” spectrum. Each spectrum was <sup>13</sup>C corrected using a software package from PC-MassSpec.

Response factors for all compound types were assumed to be 1.0, such that weight percent was determined from area percent. The acquired mass spectra were summed to generate one “averaged” spectrum. The output from the FIMS analysis is the average weight percents of alkanes, 1-unsaturations, 2-unsaturations, 3-unsaturations, 4-unsaturations, 5-unsaturations, and 6-unsaturations in the test sample.

The molecules with different numbers of unsaturations may be comprised of cycloparaffins, olefins, and aromatics. If aromatics were present in significant amounts in the lubricant

base oil they would most likely be identified in the FIMS analysis as 4-unsaturations. When olefins were present in significant amounts in the lubricant base oil they would most likely be identified in the FIMS analysis as 1-unsaturations.

5 The total of the 1-unsaturations, 2-unsaturations, 3-unsaturations, 4-unsaturations, 5-unsaturations, and 6-unsaturations from the FIMS analysis, minus the weight percent of olefins by proton NMR, and minus the weight percent of aromatics by HPLC-UV is the total weight percent of molecules with cycloparaffin functionality in the lubricant base oils of this invention. The total of the 2-unsaturations, 3-unsaturations, 4-unsaturations, 5-unsaturations, and 6-unsaturations from the FIMS analysis, minus the weight percent of aromatics by HPLC-UV is the weight percent of molecules with multicycloparaffinic functionality in the oils of this invention. Note that if the aromatics content was not measured, it was assumed to be less than 0.1 wt% and not included in the calculation for total weight percent of molecules with cycloparaffin functionality.

10 In one embodiment, the lubricant base oil fractions derived from highly paraffinic wax have a weight percent of molecules with cycloparaffinic functionality greater than 3, preferably greater than 5. Preferably, the lubricant base oil fractions derived from highly paraffinic wax also have a ratio of weight percent of molecules with monocycloparaffinic functionality to weight percent of molecules with multicycloparaffinic functionality greater than 5, preferably greater than 15, more preferably greater than 50. In a preferred embodiment, the lubricant base oil fraction comprises greater than 9 alkyl branches/100 carbons.

15 In another embodiment of the lubricant base oil fractions derived from highly paraffinic wax, there is a relationship between the weight percent of all molecules with at least one cycloparaffinic functionality and the kinematic viscosity of the lubricant base oils of this invention. That is, the higher the kinematic viscosity at 100° C. in cSt, the higher the amount of molecules with cycloparaffinic functionality that are obtained. In a preferred embodiment, the lubricant base oil fractions derived from highly paraffinic wax have a weight percent of molecules with cycloparaffinic functionality greater than the kinematic viscosity in cSt multiplied by three. The lubricant base oil fractions derived from highly paraffinic wax have a kinematic viscosity at 100° C. between about 1.0 cSt and about 3.5 cSt, preferably between about 2.0 cSt and about 3.5 cSt, and more preferably between about 2.0 cSt and about 3.0 cSt.

20 The modified ASTM D 5292-99 and HPLC-UV test methods used to measure low level aromatics, and the FIMS test method used to characterize saturates are described in D. C. Kramer, et al., “Influence of Group II & III Base Oil Composition on VI and Oxidation Stability,” presented at the 1999 AIChE Spring National Meeting in Houston, Mar. 16, 1999, 25 the contents of which is incorporated herein in its entirety.

25 Although the highly paraffinic wax feeds are essentially free of olefins, base oil processing techniques can introduce olefins, especially at high temperatures, due to ‘cracking’ reactions. In the presence of heat or UV light, olefins can 30 polymerize to form higher molecular weight products that can color the base oil or cause sediment. In general, olefins can be removed during the process of this invention by hydrofinishing or by clay treatment.

35 The properties of exemplary Fischer-Tropsch lubricant base oils suitable for use as lubricant additive diluent oils in oil soluble additive concentrates are summarized in Table II in the Examples.

## Lubricant Additives

Finished lubricants comprise at least one lubricant base oil and at least one additive. Typically, the at least one additive is added to the lubricant base oil in the form of an oil soluble additive concentrate comprising at least one additive and a lubricant additive diluent oil, to improve the additive's solubility in the lubricant base oil. The intended use for the finished lubricant will influence the additives required to provide a suitable finished lubricant.

The lubricant additive diluent oils of the present invention may be used with any additive or additive package suitable for use in lubricant base oils to provide finished lubricants.

The additives for use in lubricant base oils to provide finished lubricants include additives selected from the group consisting of viscosity index improvers, detergents, dispersants, anti-wear additives, EP agents, antioxidants, pour point depressants, viscosity index improvers, viscosity modifiers, friction modifiers, demulsifiers, antifoaming agents, colorants, color stabilizers, corrosion inhibitors, rust inhibitors, seal swell agents, metal deactivators, biocides, and mixtures thereof.

The viscosity index improvers can be selected from the group consisting of olefin copolymers, co-polymers of ethylene and propylene, polyalkylacrylates, polyalkylmethacrylates, polyisobutylene, hydrogenated styrene-isoprene copolymers, hydrogenated styrene-butadienes, and mixtures thereof.

The additives may be in the form of a lubricant additive package, which comprises several additives to provide a finished lubricant with desirable properties. Lubricant additive packages for use in lubricant base oils to provide finished lubricants include lubricant additive packages selected from the group consisting of a detergent-inhibitor (DI) package, an engine oil additive package, an automatic transmission fluid additive package, a heavy duty transmission fluid additive package, a power steering fluid additive package, a gear oil additive package, and an industrial oil additive package.

According to the present invention, the lubricant base oil fraction derived from highly paraffinic wax may be used with an engine oil additive package designed for ILSAC GF-4 or API PC-10 engine oils.

Two of the more commonly used categories of additives in finished lubricants are DI packages and VI improvers. DI packages serve to suspend oil contaminants and combustion by-products, as well as to prevent oxidation of the finished lubricant with the resultant formation of varnish and sludge deposits. VI improvers modify the viscometric characteristics of lubricants by reducing the rate of thinning with increasing temperature and the rate of thickening with low temperatures. VI improvers thereby provide enhanced performance at low and high temperatures. In many applications, VI improvers are used with DI packages to provide a finished lubricant.

## Oil Soluble Additive Concentrate

The lubricant additive diluent oils of the present invention are blended with one or more additives to provide an oil soluble additive concentrate to be added to lubricant base oil stocks to provide a finished lubricant. The oil soluble additive concentrates according to the present invention comprise the lubricant base oil fraction derived from highly paraffinic wax, as described herein, and one or more additives. The oil soluble additive concentrates according to the present invention may further comprise a conventional Group I base oil, a conventional Group II base oil, or a mixture thereof. When used as a further component in the oil soluble additive concentrates according to the present invention, preferably the conven-

tional Group I base oil or conventional Group II base oil is selected from the group consisting of 100N, 150N, 220N, and mixtures thereof.

The oil soluble additive concentrates according to the present invention are not suitable as finished lubricants on their own, but are blended with lubricant base oil stocks to provide a finished lubricant. The additives are readily soluble in the lubricant base oil fraction derived from highly paraffinic wax of the present invention, and the resulting oil soluble additive concentrates are readily soluble in lubricant base oil stocks to provide finished lubricants.

Advantageously, the oil soluble additive concentrates according to the present invention do not introduce any undesirable characteristics, including, for example, high volatility, high viscosity, high turbidity, or impurities such as heteroatoms, to the lubricant base oil stocks. The oil soluble additive concentrates according to the present invention have a low amount of heteroatom containing compounds including nitrogen and sulfur containing compounds and exhibit excellent solubility in the lubricant base oil stocks. In addition, the oil soluble additive concentrates according to the present invention exhibit good elastomer compatibility, low volatility, high oxidation stability, good low temperature properties, and low viscosity.

The oil soluble additive concentrate may be made by blending the lubricant base oil fraction derived from highly paraffinic wax and the one or more lubricant additives by techniques known to those of skill in the art. The oil soluble additive concentrate components may be blended in a single step going from the individual components (i.e., a Fischer-Tropsch derived lubricant base oil fraction, a DI package and a VI improver) directly to provide the oil soluble concentrate. In the alternative, the lubricant base oil fraction derived from highly paraffinic wax and one additive (i.e., the DI package) may be blended initially and then the resulting blend may be mixed with a second additive (i.e., the VI improver). The blend of the lubricant base oil fraction derived from highly paraffinic wax and the first additive may be isolated as such or the addition of the second additive may occur immediately.

The oil soluble additive concentrates preferably comprise 5 to 98 weight percent of the lubricant base oil fraction derived from highly paraffinic wax and at least 2 weight percent of one or more lubricant additives. More preferably, the oil soluble additive concentrates comprise 95 to 5 weight percent of the lubricant base oil fraction derived from highly paraffinic wax and 5 to 95 weight percent of one or more lubricant additives. The oil soluble additive concentrate will comprise varying amounts of the lubricant base oil fraction, used as a lubricant additive diluent oil, depending on the additive. By way of example, oil soluble additive concentrates with DI packages may contain about 50 weight % lubricant base oil fraction derived from highly paraffinic wax. Oil soluble additive concentrates with VI improver preferably comprises 2 to 20 weight % VI improver and 98 to 80 weight % lubricant base oil fraction derived from highly paraffinic wax. Oil soluble additive concentrates with gear oil additive packages may contain 25 weight % or less lubricant base oil fraction derived from highly paraffinic wax.

## Finished Lubricant

To provide finished lubricants, the oil soluble additive concentrates of the present invention are blended with one or more lubricant base oil stocks. In addition to the one or more lubricant base oil stocks, the oil soluble additive concentrates of the present invention optionally may also be blended with additional additives, other additive concentrates, or combinations thereof to provide finished lubricants. Accordingly, the finished lubricants comprise the oil soluble additive concen-

trates of the present invention and one or more lubricant base oil stocks. Optionally, the finished lubricants may also comprise additional additives, other additive concentrates, or combinations thereof.

The finished lubricant preferably comprises 0.5 to 50 weight percent of the oil soluble additive concentrates of the present invention and 30 to 99.5 weight percent of the one or more lubricant base oils, preferably 0.5 to 50 weight percent of the oil soluble additive concentrates of the present invention and 50 to 99.5 weight percent of the one or more lubricant base oils. The lubricant base oils can be any oils suitable for use as a lubricant base oil for the intended purpose of the finished lubricant. The lubricant base oils can be lubricant base oils selected from the group consisting of conventional Group I base oils, conventional Group II base oils, conventional Group III base oils, Fischer-Tropsch derived base oils, Group IV base oils, poly internal olefins, diesters, polyol esters, phosphate esters, alkylated aromatics (i.e., alkylated naphthalenes), alkylated cycloparaffins, vegetable oils, and mixtures thereof. The lubricant base oil stocks and the additives will be selected based on the intended use for the finished lubricant.

In certain embodiments, the finished lubricant according to the present invention meets the specifications for an SAE J300 multigrade engine oil. The finished lubricant according to the present invention may also meet specifications selected from the group consisting of ILSAC GF-3, ILSAC GF-4, API CI-4, API PC-10, and combinations thereof. Preferably, the finished lubricant according to the present invention comprises less than 0.7 weight % total sulfur as measured by ASTM D 1552 and more preferably less than 0.5 weight % total sulfur as measured by ASTM D 1552.

The finished lubricants may be made by blending the oil soluble additive concentrates according to the present invention with one or more lubricant base oil stocks and optionally additional additives, other additive concentrates, or combinations thereof by techniques known to those of skill in the art. The finished lubricants may be blended in a single step going from the individual components (i.e., the oil soluble additive concentrate and the one or more lubricant base oil stocks) directly to provide the finished lubricant. In the alternative, the oil soluble additive concentrate and one lubricant base oil stock may be blended initially to provide a lubricant blend and then the lubricant blend may be mixed with one or more additional lubricant base oil stocks and optionally additional additives, other additive concentrates, or combinations thereof. The lubricant blend may be isolated as such or the addition of the additional lubricant base oil stocks, additional additives, or other additive concentrates may occur immediately.

The lubricant base oil fraction derived from highly paraffinic wax used as a lubricant additive diluent oil may be manufactured at a site different from the site at which the components of the oil soluble concentrate are received and blended. In addition, the finished lubricant may be manufactured at a site different from the site at which the components of the oil soluble concentrate are received and blended.

In a preferred embodiment the lubricant base oil fraction is derived from a Fischer Tropsch process, and the oil soluble concentrate and the finished lubricant are made at the same site, which site is different from the site at which the Fischer-Tropsch derived lubricant base oil fraction is originally made. Furthermore, the components of the finished lubricant (i.e., the Fischer-Tropsch derived lubricant base oil fraction, the lubricant base oil stocks, and the additives) may all be manufactured at different sites. Preferably, the Fischer-Tropsch derived lubricant base oil fraction is manufactured at a remote

site (i.e., a location away from a refinery or market, which location may have a higher cost of construction than the cost of construction at the refinery or market. In quantitative terms, the distance of transportation between the remote site and the refinery or market is at least 100 miles, preferably more than 500 miles, and most preferably more than 1000 miles).

Preferably, the Fischer-Tropsch derived lubricant base oil is manufactured at a first remote site and shipped to a second site. The lubricant base oil stocks to be included in the finished lubricant may be manufactured at a site that is the same as the first remote site or at a third remote site. The second site receives the Fischer-Tropsch derived lubricant base oil fraction, the lubricant base oil stocks, and the additives. The oil soluble concentrate and the finished lubricant are manufactured at this second site.

#### Other Uses

In addition to use as lubricant additive diluent oils, the extra light hydrocarbon liquids of the present invention may also be used as mineral seal oil, rolling mill oil, agricultural spray oil, drilling fluid, high flash cleaning solvent, spindle oil, diluent for ink, dielectric fluid, and food grade applications.

**Drilling Fluid:** Any of a number of liquid and gaseous fluids and mixtures of fluids and solids (as solid suspensions, mixtures and emulsions of liquids, gases and solids) used in operations to drill boreholes into the earth. Classifications of drilling fluids has been attempted in many ways, often producing more confusion than insight. One classification scheme, given here, is based only on the mud composition by singling out the component that clearly defines the function and performance of the fluid: (1) water-base, (2) non-water-base and (3) gaseous (pneumatic). Each category has a variety of subcategories that overlap each other considerably. Fluids used in hydrocarbon drilling operations, especially fluids that contain significant amounts of suspended solids, emulsified water or oil. Mud includes all types of water-base, oil-base and synthetic-base drilling fluids. Drill-in, completion and workover fluids are sometimes called muds, although a fluid that is essentially free of solids is not strictly considered mud.

**Rolling Mill Oil:** A lubricant used in a machine for rolling metal into sheets, bars, or other forms. Typical metals that are rolled include steel and aluminum. The lubricant must provide a low friction coefficient, an acceptable bearing capacity, and produce a smooth product surface.

**Mineral Seal Oil:** A general term for a light lubricant having the following properties: low viscosity, light color, low odor, high aniline point, low pour point, good color stability, and low volatility.

**Agricultural Spray Oil:** A light viscosity oil sprayed on growing crops or harvested agricultural products to improve product quality and yields. They are used to reduce insect damage, control fungus and other diseases, reduce dust, and reduce evapo-transpiration. The oils must have low phytotoxicity and volatility, as well as be odorless, non-toxic, and biodegradable.

**Spindle Oil:** A light viscosity oil used in high speed lightly loaded bearings, such as those found in textile spinning frames and automated machine tools. These low viscosity oils lower operating temperatures and increases machine efficiency. They are typically formulated with additives, including anti-oxidants, rust inhibitors, and antiwear agents. Desired properties of a spindle oil are high oxidation stability, low volatility, low staining, low pour point, and high viscosity index.

**Dielectric Fluid:** Dielectric fluids are fluids that can sustain a steady electric field and act as an electrical insulator. Accordingly, dielectric fluids serve to dissipate heat gener-

ated by energizing components and to insulate those components from the equipment enclosure and from other internal parts and devices.

## EXAMPLES

The invention will be further explained by the following illustrative examples that are intended to be non-limiting.

## Example 1:

Fischer-Tropsch Wax and Preparation of  
Fischer-Tropsch Lubricant Base Oils

A sample of commercial hydrotreated Fischer-Tropsch wax made using a Fe-based Fischer-Tropsch synthesis catalyst and a sample of hydrotreated Fischer-Tropsch wax made using a Co-based Fischer-Tropsch catalyst were analyzed and found to have the properties shown in Table I.

TABLE I

|                        | Fischer-Tropsch Catalyst |          |
|------------------------|--------------------------|----------|
|                        | Fe-Based                 | Co-Based |
| Sulfur, ppm            | <6                       |          |
| Nitrogen, ppm          | 6.5*                     |          |
| Oxygen by NA, Wt %     | 0.59                     |          |
| GC N-Paraffin Analysis |                          |          |
| Total N Paraffin, Wt % | 84.47                    |          |
| Avg. Carbon Number     | 27.3                     |          |
| Avg. Molecular Weight  | 384.9                    |          |

| 5                                     |      | Fischer-Tropsch Catalyst |          |
|---------------------------------------|------|--------------------------|----------|
|                                       |      | Fe-Based                 | Co-Based |
| <u>D 6352 Sim. Dist. (Wt %), ° F.</u> |      |                          |          |
| 10                                    | 0.5  | 10                       | 515      |
|                                       | 5    | 131                      | 597      |
|                                       | 10   | 181                      | 639      |
|                                       | 20   | 251                      | 689      |
|                                       | 30   | 309                      | 714      |
|                                       | 40   | 377                      | 751      |
|                                       | 50   | 437                      | 774      |
|                                       | 60   | 497                      | 807      |
|                                       | 70   | 553                      | 839      |
|                                       | 80   | 611                      | 870      |
|                                       | 90   | 674                      | 911      |
|                                       | 95   | 707                      | 935      |
|                                       | 99.5 | 744                      | 978      |

\*duplicate tests

The Fischer-Tropsch wax feeds were hydroisomerized over a Pt/SAPO-11 catalyst on an alumina binder. Run conditions were a temperature of between 652 and 695° F. (344 and 368° C.), liquid hourly space velocity (LHSV) of 0.6 to 1.0 hr<sup>-1</sup>, 1000 psig reactor pressure, and a once-through hydrogen rate of between 6 and 7 MSCF/bbl. The reactor effluent passed directly to a second reactor, also at 1000 psig, which contained a Pt/Pd on silica-alumina hydrofinishing catalyst. Conditions in that reactor were a temperature of between 425 and 700° F. (218 and 372° C.), and LHSV of 1.0 hr<sup>-1</sup>.

The products boiling above about 600° F. were fractionated by atmospheric or vacuum distillation to produce five fractions having viscosities between about 2.0 and 3.5 cSt at 100° C. The properties of the five fractions are shown in Table II.

TABLE II

| Properties                     | Example 1 | Example 2 | Example 3 | Example 4 | Example 5 |
|--------------------------------|-----------|-----------|-----------|-----------|-----------|
| Wax Feed                       | Fe-Based  | Fe-Based  | Co-Based  | Co-Based  | Co-Based  |
| Hydroisomerization Temp, ° F.  | 681       | 681       | 694       | 671       | 690       |
| Viscosity at 100° C., cSt      | 2.981     | 2.598     | 2.583     | 2.297     | 3.189     |
| VI                             | 127       | 124       | 133       | 124       | 122       |
| Aromatics, Wt %                | 0.0128    | 0.0107    |           |           |           |
| FIMS, Wt % of Molecules        |           |           |           |           |           |
| Paraffins                      | 89.2      | 91.1      | 93.0      | 91.3      | 81.3      |
| Monocycloparaffins             | 10.8      | 8.9       | 7.0       | 8.0       | 18.7      |
| Multicycloparaffins            | 0.0       | 0.0       | 0.0       | 0.7       | 0.0       |
| Total                          | 100.0     | 100.0     | 100.0     | 100.0     | 100.0     |
| API Gravity                    | 43.4      | 44.1      | 43.85     | 44.69     |           |
| Pour Point, ° C.               | -27       | -32       | -30       | -33       | 5         |
| Cloud Point, ° C.              | -18       | -22       | -16       | -7        | 12        |
| Mono/Multicycloparaffins       | >100      | >100      | >100      | 11.4      | >100      |
| Oxidator BN, Hours             |           |           | 40.14     |           |           |
| Aniline Point, D 611-04, ° F.  | 236.5     | 226.3     |           |           |           |
| Noack Volatility, Wt %         | 32.48     | 49.18     | 48.94     |           | 21.8      |
| 160-40(Viscosity at 100° C.)   | 40.76     | 56.08     | 56.68     | 68.12     | 32.44     |
| D 6352 Sim. Dist. (Wt %), ° F. |           |           |           |           |           |
| 0.5                            | 652       | 597       | 601       | 591       | 672       |
| 5                              | 670       | 615       | 618       | 605       | 695       |
| 10                             | 681       | 626       | 630       | 616       | 707       |
| 20                             | 697       | 646       | 653       | 634       | 722       |
| 30                             | 713       | 666       | 673       | 652       | 734       |
| 40                             | 728       | 686       | 693       | 668       | 744       |
| 50                             | 744       | 706       | 713       | 684       | 755       |
| 60                             | 760       | 726       | 733       | 699       | 767       |
| 70                             | 776       | 748       | 754       | 715       | 779       |
| 80                             | 792       | 769       | 777       | 732       | 793       |
| 90                             | 808       | 791       | 802       | 750       | 810       |
| 95                             | 817       | 803       | 816       | 767       | 823       |

TABLE II-continued

| Properties                                 | Example 1    | Example 2    | Example 3         | Example 4   | Example 5   |
|--------------------------------------------|--------------|--------------|-------------------|-------------|-------------|
| 95.5<br>NMR, Alkyl Branches/100<br>Carbons | 833<br>10.05 | 825<br>10.36 | 833<br>Not tested | 800<br>9.46 | 850<br>9.20 |

## Example 2:

## Preparation of Oil Soluble Additive Concentrates

The above-example five Fischer-Tropsch derived lubricant base oil fractions can be used as lubricant additive diluent oils and blended with additives to provide an oil soluble additive concentrate. 15

As such, 98 to 80 weight percent Fischer-Tropsch derived lubricant base oil fraction is blended with 20 to 2 weight percent olefin copolymer VI improver to provide oil soluble additive concentrates. By way of example, Example 3 Fischer-Tropsch derived lubricant base oil fraction was blended with approximately 6 weight percent olefin copolymer VI improver. There was no evidence of polymer coming out of solution or of any other gross insolubility. 20

## Example 3:

## Comparative Example

The properties of four commercially available conventional petroleum-derived oils (Pennzoil 75HC, Petro Canada VHV12, Nexbase 3020, and Ergon Hygold 60) and a commercially available polyalphaolefin (Chevron Synfluid 2) having viscosities below 3.0 cSt at 100° C. are shown in Table III. 30

TABLE III

|                                 | Pennzoil<br>75HC | Petro<br>Canada<br>VHV12 | Nexbase<br>3020 | Ergon<br>Hygold 60 | Chevron<br>Synfluid 2 |
|---------------------------------|------------------|--------------------------|-----------------|--------------------|-----------------------|
| Viscosity at<br>100° C.,<br>cSt | 2.885            | 2.434                    | 2.055           | 2.265              | 1.726                 |
| VI                              | 80               | 103                      | 96              | 36                 | 146                   |
| Pour Point,<br>° C.             | -38              | -42                      | -51             | -61                | Not<br>tested         |
| Noack<br>Volatility,<br>Wt %    | 59.1             | 69.5                     | 70              | 98.5               | 99.9                  |

The above-exemplified conventional petroleum-derived oils and polyalphaolefin having viscosities between 2.0 and 3.5 cSt at 100° C. all have Noack volatilities greater than 50 weight percent, and more specifically greater than 59 weight percent. In comparison, the Noack volatilities of the Fischer-Tropsch lubricant base oil fractions of Examples 1-5 were all significantly less than 50 weight percent. Accordingly, the Fischer-Tropsch lubricant base oil fractions of the present invention have low volatility and low viscosity. 55

While the present invention has been described with reference to specific embodiments, this application is intended to cover those various changes and substitutions that may be made by those of ordinary skill in the art without departing from the spirit and scope of the appended claims. 65

What is claimed is:

1. A lubricant additive diluent oil comprising: a lubricant base oil fraction having a viscosity of between about 1.0 and 3.0 cSt at 100° C. and a Noack volatility of less than a Noack Volatility Factor as calculated by the following equation: Noack Volatility Factor = 160 - 40 (Kinematic Viscosity at 100° C.), wherein the lubricant base oil fraction comprises greater than 3 weight % molecules with cycloparaffinic functionality and less than 0.30 weight percent aromatics and comprises greater than 9 alkyl branches/100 carbons and has a ratio of weight % of molecules with monocycloparaffinic functionality to weight % of molecules with multicycloparaffinic functionality of greater than 15. 10
2. The lubricant additive diluent oil of claim 1, wherein the lubricant base oil fraction is a Fischer-Tropsch derived lubricant base oil fraction. 15
3. The lubricant additive diluent oil of claim 1, wherein the lubricant base oil fraction comprises greater than 5 weight % molecules with cycloparaffinic functionality. 20
4. The lubricant additive diluent oil of claim 1, wherein the lubricant base oil fraction comprises a ratio of weight % of molecules with monocycloparaffinic functionality to weight % of molecules with multicycloparaffinic functionality of greater than 50. 25
5. The lubricant additive diluent oil of claim 1, wherein the lubricant base oil fraction comprises a weight % of molecules with cycloparaffinic functionality of greater than the kinematic viscosity at 100° C. multiplied by three. 30
6. The lubricant additive diluent oil of claim 1, wherein the lubricant base oil fraction has a Noack volatility of less than 50 weight %. 35
7. The lubricant additive diluent oil of claim 1, wherein the lubricant additive diluent oil further comprises a conventional Group I base oil or a conventional Group II base oil. 40
8. An oil soluble additive concentrate comprising: 45
- 5 to 98 weight % of a lubricant base oil fraction having a viscosity of between about 1.0 and 3.0 cSt at 100° C. and a Noack volatility of less than a Noack Volatility Factor as calculated by the following equation: Noack Volatility Factor = 160 - 40 (Kinematic Viscosity at 100° C.), wherein the lubricant base oil fraction comprises greater than 3 weight % molecules with cycloparaffinic functionality and less than 0.30 weight percent aromatics and comprises greater than 9 alkyl branches/100 carbons and has a ratio of weight % of molecules with monocycloparaffinic functionality to weight % of molecules with multicycloparaffinic functionality of greater than 15; and 50
- at least 2 weight % of one or more lubricant additives. 55
9. The oil soluble additive concentrate of claim 8, wherein the lubricant base oil fraction is a Fischer-Tropsch derived lubricant base oil fraction. 60
10. The oil soluble additive concentrate of claim 8, wherein the lubricant base oil fraction has a viscosity between about 2.0 and 3.0 cSt at 100° C. 65
11. The oil soluble additive concentrate of claim 10, wherein the lubricant base oil fraction has a viscosity index of between about 105 and 155. 65

## 31

12. The oil soluble additive concentrate of claim 8, wherein the lubricant base oil fraction has a Viscosity Index greater than a Viscosity Index Factor as calculated by the following equation:

Viscosity Index Factor =  $28 \times \ln(\text{Kinematic Viscosity of the Fischer-Tropsch derived lubricant base oil fraction at } 100^\circ \text{ C.}) + 95$ . 5

13. The oil soluble additive concentrate of claim 8, wherein the lubricant base oil fraction comprises a weight % of molecules with cycloparaffinic functionality of greater than the kinematic viscosity at  $100^\circ \text{ C.}$  multiplied by three. 10

14. The oil soluble additive concentrate of claim 8, wherein the lubricant base oil fraction has a Noack volatility of less than 50 weight %. 15

15. The oil soluble additive concentrate of claim 8, wherein the oil soluble additive concentrate further comprises a conventional Group I base oil or a conventional Group II base oil. 15

16. The oil soluble additive concentrate of claim 8, wherein the lubricant base oil fraction has an aniline point greater than  $36 \times \ln(\text{Kinematic Viscosity of the lubricant base oil fraction at } 100^\circ \text{ C.}) + 200$ . 20

17. The oil soluble additive concentrate of claim 8, wherein the lubricant base oil fraction comprises greater than 5 weight % molecules with cycloparaffinic functionality. 25

18. The oil soluble additive concentrate of claim 8, wherein the lubricant base oil fraction comprises a ratio of weight % of molecules with monocycloparaffinic functionality to weight % of molecules with multicycloparaffinic functionality of greater than 50. 25

19. The oil soluble additive concentrate of claim 8, wherein the lubricant base oil fraction has a sulfur content of less than 5 ppmw. 30

20. The oil soluble additive concentrate of claim 8, wherein the one or more lubricant additives are selected from the group consisting of viscosity index improvers, detergents, dispersants, anti-wear additives, EP agents, antioxidants, pour point depressants, viscosity index improvers, viscosity modifiers, friction modifiers, demulsifiers, antifoaming agents, colorants, color stabilizers, corrosion inhibitors, rust inhibitors, seal swell agents, metal deactivators, biocides, and mixtures thereof. 35

21. The oil soluble additive concentrate of claim 8, wherein the one or more lubricant additives comprise a lubricant additive package. 40

22. The oil soluble additive concentrate of claim 21, wherein the lubricant additive package is selected from the group consisting of a detergent-inhibitor package, an engine oil additive package, an automatic transmission fluid additive package, a heavy duty transmission fluid additive package, a power steering fluid additive package, a gear oil additive package, and an industrial oil additive package. 45

23. The oil soluble additive concentrate of claim 20, wherein the oil soluble additive concentrate comprises 2 – 20 weight % viscosity index improver. 50

24. The oil soluble additive concentrate of claim 23, wherein the viscosity index improver is selected from the group consisting of olefin copolymers, co-polymers of ethylene and propylene, polyalkylacrylates, polyalkylmethacrylates, polyisobutylene, hydrogenated styrene-isoprene copolymers, hydrogenated styrene-butadienes, and mixtures thereof. 55

25. A finished lubricant comprising:

a. an oil soluble additive concentrate comprising:

- i. 5 to 98 weight % of a lubricant base oil fraction having a viscosity of between about 1.0 and 3.0 cSt at  $100^\circ \text{ C.}$  and a Noack volatility of less than a Noack Volatility Factor as calculated by the following equation:

## 32

Noack Volatility Factor =  $160 - 40(\text{Kinematic Viscosity at } 100^\circ \text{ C.})$ , wherein the lubricant base oil fraction comprises greater than 3 weight % molecules with cycloparaffinic functionality and less than 0.30 weight percent aromatics and comprises greater than 9 alkyl branches/100 carbons and has a ratio of weight % of molecules with monocycloparaffinic functionality to weight % of molecules with multicycloparaffinic functionality of greater than 15; and 5

ii. at least 2 weight % of one or more lubricant additives; and 10

b. one or more lubricant base oils. 15

26. The finished lubricant of claim 25, wherein the finished lubricant comprises 0.5 to 50 weight % oil soluble additive concentrate and 30 to 99.5 weight % one or more lubricant base oils. 20

27. The finished lubricant of claim 25, wherein the lubricant base oil fraction comprises greater than 5 weight % molecules with cycloparaffinic functionality. 25

28. The finished lubricant of claim 25, wherein the lubricant base oil fraction comprises a ratio of weight % of molecules with monocycloparaffinic functionality to weight % of molecules with multicycloparaffinic functionality of greater than 50. 30

29. The finished lubricant of claim 25, wherein the lubricant base oil fraction has a Noack volatility of less than 50 weight %. 35

30. The finished lubricant of claim 25, wherein the oil soluble additive concentrate further comprises a conventional Group I base oil or a conventional Group II base oil. 40

31. The finished lubricant of claim 25, wherein the one or more lubricant additives are selected from the group consisting of viscosity index improvers, detergents, dispersants, anti-wear additives, EP agents, antioxidants, pour point depressants, viscosity index improvers, viscosity modifiers, friction modifiers, demulsifiers, antifoaming agents, colorants, color stabilizers, corrosion inhibitors, rust inhibitors, seal swell agents, metal deactivators, biocides, and mixtures thereof. 45

32. The finished lubricant of claim 25, wherein the one or more lubricant additives comprise a lubricant additive package. 50

33. The finished lubricant of claim 32, wherein the lubricant additive package is selected from the group consisting of a detergent-inhibitor package, an engine oil additive package, an automatic transmission fluid additive package, a heavy duty transmission fluid additive package, a power steering fluid additive package, a gear oil additive package, and an industrial oil additive package. 55

34. The finished lubricant of claim 25, wherein the one or more lubricant base oils are selected from the group consisting of conventional Group I base oils, conventional Group II base oils, conventional Group III base oils, Fischer-Tropsch derived base oils, Group IV base oils, poly internal olefins, diesters, polyol esters, phosphate esters, alkylated aromatics, alkylated cycloparaffins, alkylated naphthalenes, vegetable oils, and mixtures thereof. 60

35. The finished lubricant of claim 25, wherein the finished lubricant meets the specifications for an SAE J300 multigrade engine oil. 65

36. The finished lubricant of claim 35, wherein the finished lubricant further meets specifications selected from the group consisting of ILSAC GF-3, ILSAC GF-4, API CI-4, API PC-10, and combinations thereof. 70

37. The finished lubricant of claim 25, wherein the finished lubricant comprises less than 0.7 weight % total sulfur as measured by ASTM D 1552. 75

**33**

**38.** The lubricant additive diluent oil of claim 1, wherein the lubricant base oil fraction comprises greater than 10 alkyl branches/100 carbons.

**39.** The oil soluble additive concentrate of claim 8, wherein the lubricant base oil fraction comprises greater than 10 alkyl branches/100 carbons.

**40.** The finished lubricant of claim 25, wherein the lubricant base oil fraction comprises greater than 10 alkyl branches/100 carbons.

**41.** The oil soluble additive concentrate of claim 22, 10 wherein the lubricant additive package is a detergent-inhibi-

**34**

tor package and the oil soluble additive concentrate comprises about 50 weight percent lubricant base oil fraction.

**42.** The oil soluble additive concentrate of claim 22, wherein the lubricant additive package is a gear oil additive package and the oil soluble additive concentrate comprises about 25 weight percent or less lubricant base oil fraction.

**43.** The finished lubricant of claim 26, wherein the oil soluble additive concentrate comprises 50 weight % or more lubricant additives.

\* \* \* \* \*